



US005338471A

**United States Patent** [19]

Lal

[11] **Patent Number:** **5,338,471**[45] **Date of Patent:** **Aug. 16, 1994**

[54] **POUR POINT DEPRESSANTS FOR INDUSTRIAL LUBRICANTS CONTAINING MIXTURES OF FATTY ACID ESTERS AND VEGETABLE OILS**

[75] Inventor: **Kasturi Lal**, Willoughby, Ohio

[73] Assignee: **The Lubrizol Corporation**, Wickliffe, Ohio

[21] Appl. No.: **137,445**

[22] Filed: **Oct. 15, 1993**

[51] Int. Cl.<sup>5</sup> ..... **C10M 141/02**

[52] U.S. Cl. ..... **252/56 S; 252/56 R;**

**252/51.5 A; 252/32.7 E; 252/50; 252/47;**  
**252/52 R; 44/403**

[58] Field of Search ..... **252/51.5 A, 56 S, 56 R,**  
**252/32.7 E, 47, 50, 52; 44/403**

[56] **References Cited**

**U.S. PATENT DOCUMENTS**

- |           |         |                 |                |
|-----------|---------|-----------------|----------------|
| 2,243,198 | 5/1941  | Dietrich        | ..... 44/8     |
| 2,345,579 | 4/1944  | Buxton          | ..... 44/66    |
| 2,978,395 | 4/1961  | Hollyday et al. | ..... 204/154  |
| 3,147,222 | 9/1964  | Bauer           | ..... 252/51.5 |
| 3,288,577 | 11/1966 | Patinkin et al. | ..... 44/62    |
| 3,304,260 | 2/1967  | Fields et al.   | ..... 252/51.5 |
| 3,449,250 | 6/1969  | Fields          | ..... 252/51.5 |
| 3,961,915 | 6/1976  | Wisotsky        | ..... 44/62    |

- |           |         |                |                |
|-----------|---------|----------------|----------------|
| 4,364,743 | 12/1982 | Erner          | ..... 44/66    |
| 4,391,721 | 7/1983  | Pappas         | ..... 252/51.5 |
| 4,575,382 | 3/1986  | Sweeney et al. | ..... 44/57    |
| 4,604,221 | 8/1986  | Bryant et al.  | ..... 252/51.5 |
| 4,695,411 | 9/1987  | Stern et al.   | ..... 44/403   |
| 4,753,743 | 6/1988  | Seck           | ..... 252/56 S |
| 4,783,274 | 11/1988 | Jokinen et al. | ..... 252/56 S |
| 4,885,104 | 12/1989 | Sturwold       | ..... 252/56 S |
| 4,921,624 | 5/1990  | Kammann, Jr.   | ..... 252/56 S |
| 5,034,144 | 7/1991  | Ohgake et al.  | ..... 252/56 S |
| 5,160,506 | 11/1992 | Chur et al.    | ..... 44/308   |

*Primary Examiner*—Jacqueline V. Howard

*Attorney, Agent, or Firm*—James L. Cordek; Frederick D. Hunter, Sr.; Joseph P. Fischer

[57] **ABSTRACT**

This invention relates to a composition containing the combination of:

- (A) at least one vegetable or synthetic triglyceride,
- (B) esters from the transesterification of at least one animal or vegetable oil triglyceride,
- (C) a pour point depressant, and
- (D) a performance additive.

The composition may optionally contain

- (E) other oils.

**69 Claims, No Drawings**

**POUR POINT DEPRESSANTS FOR INDUSTRIAL  
LUBRICANTS CONTAINING MIXTURES OF  
FATTY ACID ESTERS AND VEGETABLE OILS**

**FIELD OF THE INVENTION**

The present invention relates to vegetable oils that possess at least 60 percent monounsaturation content, vegetable oils that are transesterified and contain at least one pour point depressant. In addition to pour point depressants, the vegetable oil and transesterified product also contains a performance additive designed to enhance the performance of the vegetable oil and transesterified product when used in hydraulic fluids, two-cycle (two stroke) internal combustion engines, gear oils, and passenger car motor oils.

The product of this invention has utility as a lubricant. Lubricants can be classified into two broad categories, engine and non-engine lubricants. Further breakdown of these two classes is given below.

**Engine Lubricants**

1. Gasoline engine oils
2. Diesel engine oils
  - Automotive diesel oils
  - Stationary diesel oils
  - Railroad diesel oils
  - Marine diesel oils
3. Natural gas engine oils
4. Aviation engine oils
5. Two-stroke cycle engine oils

**Non-Engine Lubricants**

1. Transmission fluids
  - Automatic transmission fluids
  - Manual transmission fluids
  - Power transmission fluids
2. Power steering fluids
3. Shock absorber fluids
4. Gear oils
  - Automotive gear oils
  - Industrial gear oils
5. Hydraulic fluids
  - Tractor hydraulic fluids
  - Industrial hydraulic fluids
6. Metalworking fluids
7. Miscellaneous industrial oils
8. Greases

**BACKGROUND OF THE INVENTION**

Successful use of esters of transesterified natural oils in combination with high monounsaturation vegetable oils as environmentally friendly, that is biodegradable, base fluids in industrial applications and also as a fuel additive when mixed with normally liquid fuels, is contingent upon improving their low temperature viscosities. For example, a methyl ester obtained from the transesterification of rapeseed oil, has utility as an environmentally friendly diesel fuel. However, this methyl ester has a pour point of  $-12^{\circ}\text{C}$ . and solidifies at  $13.6^{\circ}\text{C}$ . which results in clogged filters and engine failure. A sunflower oil containing an oleic acid content of 80 percent has a pour point of  $-12^{\circ}\text{C}$ . and also solidifies. Many of the industrial applications require a pour point of less than  $-25^{\circ}\text{C}$ . and a Brookfield viscosity of 7500 to 110,000 centipoises (cP) at  $-25^{\circ}\text{C}$ . In order to take advantage of the biodegradability of transesterified esters of natural oils in combination with high monoun-

saturation vegetable oils it becomes necessary to lower the pour point.

U.S. Pat. No. 2,243,198 (Dietrich, May 27, 1941) relates to non-viscous normally liquid hydrocarbon oils and more particularly to the production of fuel oils having improved flow characteristics under low temperature conditions. The flow characteristics of fuel oil is improved by the addition of a hydrogenated castor oil derivative to a non-viscous normally liquid hydrocarbon oil. Hydrogenated castor oil derivative is defined as the product obtained by reacting hydrogenated castor oil either with its own hydroxyl group or with another organic compound selected from the classes of alcohols, aldehydes, acids, isocyanates and isothiocyanates.

U.S. Pat. No. 3,598,736 (Van der Meij et al, Aug. 10, 1971) relates to soluble polyalkylmethacrylates which can be used in lubricating oil compositions to reduce the pour point. Within the polyalkylmethacrylate the alkyl group has from 10-20 carbon atoms and meets the following three requirements:

- (1) The average number of carbon atoms of the alkyl chains in the methacrylates is between 13.8 and 14.8.
- 25 (2) The molar percentage of the alkyl methacrylates with branched alkyl chains is between 10 and 30.
- (3) The molar percentage of the alkyl methacrylates with an odd number of carbon atoms in the alkyl chain is between 20 and 50.
- 30 These polymers are capable not only of considerably depressing the pour point of light lubricating oils, such a spindle oil and light machine oil, but show in addition a high activity as pour point depressants in heavy lubricating oils rich in residual components, such as heavy machine oil.

U.S. Pat. No. 3,702,300 (Coleman, Nov. 7, 1972) relates to a carboxy-containing interpolymer in which some of the carboxy radicals are esterified and the remaining carboxy radicals are neutralized by reaction with a polyamine compound having one primary or secondary amino group and is useful as an additive in lubricating compositions and fuels. The interpolymer is especially effective to impart desirable viscosity characteristics and anti-sludge properties to a lubricating oil.

U.S. Pat. No. 4,284,414 (Bryant, Aug. 18, 1981) relates to the use of mixed alkyl esters made by reacting two or more of certain monohydric alcohols with interpolymers which contain units derived from (i)  $\alpha,\beta$ -unsaturated dicarboxylic acids, or derivatives thereof and (ii) vinyl aromatic monomers having up to 12 carbon atoms in crude oils. Minor amounts of the mixed alkyl esters are useful for modifying the fluidity and flow characteristics of crude oils, and more particularly, for improving the pipeline pumpability of crude oils.

U.S. Pat. No. 4,364,743 (Erner, Dec. 21, 1982) relates to a fuel source for oil burning devices which is a fuel in and of itself or can be mixed with petroleum middle distillates. Fatty acids of the formula



65 can provide such a fuel wherein

- (a) R is (1) an alkyl radical having from 1 to 12 carbon atoms, (2) alkoxy alkyl wherein the alkoxy portion has from 1 to 4 carbon atoms and the alkyl portion

## DETAILED DESCRIPTION OF THE INVENTION

- is ethyl or propyl, (3) cyclopentyl or cyclohexyl and (4) hydroxy ethyl and hydroxy propyl;  
 (b)  $n=11-22$ ;  
 (c)  $a=2n+1, 2n-1, 2n-3, 2n-5$ , or  $2n-7$ ; and  
 (d)  $x$  is 0 or 1.

U.S. Pat. No. 4,575,382 (Sweeney et al, Mar. 11, 1986) relates to a vegetable oil containing middle distillate fuel characterized by an improved thermal stability. The vegetable oils which may be used include soybean oil, peanut oil and sunflower seed oil.

U.S. Pat. No. 4,695,411 (Stem et al, Sep. 22, 1987) relates to a process for manufacturing a major portion of ethyl esters usable as gas oil substitute motor fuel by transesterification of an animal or vegetable oil optionally containing free acids.

U.S. Pat. No. 4,767,551 (Hunt et al, Aug. 30, 1988) relates to overbased copper-containing lubricant compositions with improved stability and antiwear and antirust properties wherein the overbased copper-containing composition inhibits the oxidation of the lubricant and preserves the antirust properties of the lubricant without significantly decreasing the antiwear properties of the zinc dialkyldithiophosphate antiwear additive during use of the lubricant in an operating engine. Further, this reference provides lubricating oil compositions containing a lubricating oil, a dispersant, a viscosity index improver dispersant, an antiwear agent and a dispersant/detergent, antioxidant and rust inhibitor comprising an overbased copper-containing composition which provides an improved lubricating oil formulation for high speed, high temperature gasoline and diesel engine operation.

U.S. Pat. No. 4,783,274 (Jokinen et al, Nov. 8, 1988) is concerned with an anhydrous oily lubricant, which is based on vegetable oils, which is substituted for mineral lubricant oils, and which, as its main component, contains triglycerides that are esters of saturated and/or unsaturated straight-chained C<sub>10</sub> to C<sub>22</sub> fatty acids and glycerol. The lubricant is characterized in that it contains at least 70 percent by weight of a triglyceride whose iodine number is at least 50 and no more than 125 and whose viscosity index is at least 190. As its basic component, instead of or along with the said triglyceride, the lubricant oil may also contain a polymer prepared by hot-polymerization out of the said triglyceride or out of a corresponding triglyceride. As additives, the lubricant oil may contain solvents, fatty acid derivatives, in particular, their metal salts, organic or inorganic, natural or synthetic polymers, and customary additives for lubricants.

U.S. Pat. No. 5,160,506 (Schur et al, Nov. 3, 1992) relates to a liquid fuel mixture, comprising a C<sub>3</sub> and/or at least a C<sub>4</sub>-alkane, at least one oil component and optionally at least one additive, a process for its preparation and its use for two-stroke engines.

## SUMMARY OF THE INVENTION

This invention relates to a composition containing the combination of:

- (A) at least one vegetable or synthetic triglyceride,
- (B) esters from the transesterification of at least one animal or vegetable oil triglyceride,
- (C) a pour point depressant, and
- (D) a performance additive.

The composition may optionally contain

- (E) other oils.

5 In practicing this invention a triglyceride oil is employed which is a natural or synthetic oil of the formula



wherein R<sup>1</sup>, R<sup>2</sup> and R<sup>3</sup> are aliphatic hydrocarbyl groups having at least 60 percent monounsaturated character and containing from about 6 to about 24 carbon atoms. The term "hydrocarbyl group" as used herein denotes a radical having a carbon atom directly attached to the remainder of the molecule. The aliphatic hydrocarbyl groups include the following:

- (1) Aliphatic hydrocarbon groups; that is, alkyl groups such as heptyl, nonyl, undecyl, tridecyl, heptadecyl; alkenyl groups containing a single double bond such as heptenyl, nonenyl, undecenyl, tridecenyl, heptadecenyl, heneicosenyl; alkenyl groups containing 2 or 3 double bonds such as 8,11-heptadecadienyl and 8,11,14-heptadecatrienyl. All isomers of these are included, but straight chain groups are preferred.
- (2) Substituted aliphatic hydrocarbon groups; that is groups containing non-hydrocarbon substituents which, in the context of this invention, do not alter the predominantly hydrocarbon character of the group. Those skilled in the art will be aware of suitable substituents; examples are hydroxy, carbalkoxy, (especially lower carbalkoxy) and alkoxy (especially lower alkoxy), the term, "lower" denoting groups containing not more than 7 carbon atoms.

- (3) Hetero groups; that is, groups which, while having predominantly aliphatic hydrocarbon character within the context of this invention, contain atoms other than carbon present in a chain or ring otherwise composed of aliphatic carbon atoms. Suitable hetero atoms will be apparent to those skilled in the art and include, for example, oxygen, nitrogen and sulfur.

Naturally occurring triglycerides are vegetable oil triglycerides. The synthetic triglycerides are those formed by the reaction of one mole of glycerol with three moles of a fatty acid or mixture of fatty acids. Preferred are vegetable oil triglycerides.

Regardless of the source of the triglyceride oil, the fatty acid moieties are such that the triglyceride has a monounsaturated character of at least 60 percent, preferably at least 70 percent and most preferably at least 80 percent. Normal sunflower oil has an oleic acid content of 25-30 percent. By genetically modifying the seeds of sunflowers, a sunflower oil can be obtained wherein the oleic content is from about 60 percent up to about 90 percent. For example, a triglyceride comprised exclusively of an oleic acid moiety has an oleic acid content of 100% and consequently a monounsaturated content of 100%. Where the triglyceride is made up of acid

moieties that are 70% oleic acid, 10% stearic acid, 5% palmitic acid, 7% linoleic and 8% hexadecanoic acid, the monounsaturated content is 78%. It is also preferred that the monounsaturated character be derived from an oleyl radical, i.e.,



is the residue of oleic acid. The preferred triglyceride oils are high oleic (at least 60 percent) acid triglyceride oils. Typical high oleic vegetable oils employed within the instant invention are high oleic safflower oil, high oleic corn oil, high oleic rapeseed oil, high oleic sunflower oil, high oleic soybean oil, high oleic cottonseed oil and high oleic palm olein. A preferred high oleic vegetable oil is high oleic sunflower oil obtained from *Helianthus* sp. This product is available from SVO Enterprises Eastlake, Ohio as Sunyl® high oleic sunflower oil. Sunyl 80 is a high oleic triglyceride wherein the acid moieties comprise 80 percent oleic acid. Another preferred high oleic vegetable oil is high oleic rapeseed oil obtained from *Brassica campestris* or *Brassica napus*, also available from SVO Enterprises as RS® high oleic rapeseed oil. RS80 signifies a rapeseed oil wherein the acid moieties comprise 80 percent oleic acid.

(B) The Transesterified Esters

The transesterified ester is formed by reacting a natural oil comprising animal fat or vegetable oils with an alcohol. These natural oils are triglycerides of the formula



wherein  $\text{R}^1$ ,  $\text{R}^2$  and  $\text{R}^3$  are as defined for component (A).

Animal fats having utility are beef tallow oil and menhaden oil. Useful vegetable oils are sunflower oil, cottonseed oil, safflower oil, corn oil, soybean oil, rapeseed oil, meadowfoam oil or any of the previously mentioned vegetable oils within component (A) that are genetically modified such that the monounsaturated content is greater than the normal value.

Alcohols utilized in forming the transesterified esters are of the formula  $\text{R}^4\text{OH}$  wherein  $\text{R}^4$  is an aliphatic group that contains from 1 to about 24 carbon atoms. The  $\text{R}^4$  may be straight chained or branched chain, saturated or unsaturated. An illustrative but non exhaustive list of alcohols are: methyl alcohol, ethyl alcohol, n-propyl alcohol, isopropyl alcohol and the isomeric butyl, pentyl, hexyl, heptyl, octyl, nonyl, dodecyl, pentadecyl and octadecyl alcohols. Preferably the alcohol is methyl alcohol.

The transesterification occurs by mixing at least 3 moles of  $\text{R}^4\text{OH}$  per 1 mole of triglyceride. A catalyst, when employed, comprises alkali or alkaline earth metal alkoxides containing from 1 up to 6 carbon atoms. Preferred catalysts are sodium or potassium methoxide, calcium or magnesium methoxide, the ethoxides of sodium, potassium, calcium or magnesium and the isomeric propoxides of sodium, potassium, calcium or

magnesium. The most preferred catalyst is sodium methoxide. The transesterification occurs at a temperature of from ambient up to the decomposition temperature of any reactant or product. Usually the upper temperature limit is not more than 150° C. and preferably not more than 120° C. In the transesterification mixed esters are obtained according to the following reaction:



25 Transesterification is an equilibrium reaction. To shift the equilibrium to the right it is necessary to use either a large excess of alcohol, or else remove glycerol as it is formed. When using an excess of alcohol, once the transesterification reaction is complete the excess alcohol is removed by distillation.

The following examples are illustrative of the preparation of the transesterified product of the present invention. Unless otherwise indicated, all parts and percentages are by weight.

35

EXAMPLE B-1

Charged to a 12 liter 4 neck flask is 7056 parts (8 moles) high oleic (80%) rapeseed oil, 1280 parts (40 moles) absolute methyl alcohol and 70.5 parts (1.30 moles) sodium methoxide. The contents are heated to a reflux temperature of 73° C. and held at this temperature for 3 hours and 76 parts (0.65 moles) of 85% phosphoric acid is added dropwise in 0.4 hours to neutralize the catalyst. Excess methyl alcohol is then removed by heating to 100° C. with nitrogen blowing at 0.2 cubic feet per hour and later to a vacuum of 30 millimeters of mercury. The contents are filtered to give 6952 parts of the transesterified methyl ester of high oleic rapeseed oil.

50

EXAMPLE B-2

The procedure of Example B-1 is essentially followed except that the high oleic rapeseed oil is replaced with high oleic (80%) sunflower oil to give the transesterified methyl ester of high oleic sunflower oil.

55

EXAMPLE B-3

Charged to a 5 liter 4 neck flask is 759 parts (12.5 moles) isopropyl alcohol. While at room temperature, 5.75 parts (0.25 moles) elemental sodium is slowly added. When all the sodium is reacted, added is 2205 (2.5 moles) high oleic (80%) sunflower oil. The contents are heated to 85° C. and held for 4 hours followed by neutralization of the catalyst with 9.67 parts (0.083 moles) of 85% phosphoric acid. The contents are stripped to 120° C. at 27 millimeters of mercury to give 2350 parts of the transesterified isopropyl ester of high oleic sunflower oil.

## EXAMPLE B-4

The procedure of Example B-3 is essentially followed except that the catalyst is made by reacting 690 parts (15 moles) absolute ethyl alcohol with 6.9 parts (0.3 moles) sodium metal and then followed by the addition of 2646 parts (3.0 moles) high oleic (80%) sunflower oil. The catalyst is neutralized with 11.6 parts (0.10 moles) of 85% phosphoric acid. The product obtained is the transesterified ethyl ester of high oleic sunflower oil.

## EXAMPLE B-5

The procedure of Example B-4 is essentially followed except that the catalyst is made by reacting 910 parts (15 moles) n-propyl alcohol with 6.9 parts (0.3 moles) sodium metal. The product obtained is the transesterified n-propyl ester of high oleic sunflower oil.

## EXAMPLE B-6

The procedure of Example B-4 is followed except that the catalyst is made by reacting 1114.5 parts (15 moles) n-butyl alcohol with 6.9 parts (0.3 moles) sodium metal. The product obtained is the transesterified n-butyl ester of high oleic sunflower oil.

## EXAMPLE B-7

The procedure of Example B-3 is essentially followed except that the catalyst is made by reacting 1300 (12.5 moles) n-hexyl alcohol with 5.75 parts (0.25 moles) sodium metal and then followed by the addition of 2205 parts (2.5 moles) high oleic (80%) sunflower oil. The catalyst is neutralized with 9.7 parts (0.083 moles) of 85% phosphoric acid. The product obtained is the transesterified n-hexyl ester of high oleic sunflower oil.

## EXAMPLE B-8

Utilizing the catalyst as prepared in Example B-3, safflower oil is transesterified with isopropyl alcohol to obtain transesterified isopropyl esters of safflower oil.

## EXAMPLE B-9

Utilizing the catalyst as prepared in Example B-4, cottonseed oil is transesterified with ethyl alcohol to obtain transesterified ethyl esters of cottonseed oil.

## EXAMPLE B-10

Utilizing the catalyst as prepared in Example B-6, corn oil is transesterified with n-butyl alcohol to obtain transesterified n-butyl esters of corn oil.

## EXAMPLE B-11

The procedure of Example B-9 is essentially followed except that beef tallow oil is utilized instead of cottonseed oil. The product obtained is the transesterified 55 ethyl ester of beef tallow oil.

## EXAMPLE B-12

The procedure of Example B-10 is essentially followed except that menhaden oil is utilized instead of corn oil. The product obtained is the transesterified 60 n-butyl ester of menhaden oil.

## EXAMPLE B-13

The procedure of Example B-1 is essentially followed except that rapeseed oil is utilized instead of high oleic rapeseed oil. The product obtained is the transesterified 65 methyl ester of rapeseed oil.

## EXAMPLE B-14

The procedure of Example B-1 is essentially followed except that soybean oil is utilized instead of high oleic rapeseed oil. The product obtained is the transesterified methyl ester of soybean oil.

## (C) The Pour Point Depressant

A drawback of using transesterified esters in combination with high monounsaturation vegetable oils is in the difficulty with congelation of this mixture at low temperatures (less than -10° C.). This difficulty arises from a natural stiffening at low temperatures of the transesterified esters and high monounsaturation vegetable oils analogous to the stiffening of honey or molasses at a reduced temperature. To maintain the "pour" or "flow" of this mixture, a pour point depressant is added to the oil.

Pour point depressants (PPD) having utility in this invention are carboxy containing interpolymers in which many of the carboxy groups are esterified and the remaining carboxy groups, if any, are neutralized by reaction with amino compounds; acrylate polymers, nitrogen containing acrylate polymers and methylene linked aromatic compounds.

## 25 Carboxy-Containing Interpolymers

This PPD is an ester of a carboxy-containing interpolymer, said interpolymer having a reduced specific viscosity of from about 0.05 to about 2, said ester being substantially free of titratable acidity, i.e., at least 90% esterification, and being characterized by the presence within its polymeric structure of pendant polar groups: (A) a relatively high molecular weight carboxylic ester group having at least 8 aliphatic carbon atoms in the ester radical, (B) a relatively low molecular weight carboxylic ester group having no more than 7 aliphatic carbon atoms in the ester radical, and optionally (C) a carbonyl-polyamino group derived from a polyamino compound having one primary or secondary amino group, wherein the molar ratio of (A):(B) is (1-20):1, preferably (1-10):1 and wherein the molar ratio of (A):(B):(C) is

(50-100):(5-50):(0.1-15)

45 An essential element of this ester is that the ester is a mixed ester, i.e., one in which there is the combined presence of both a high molecular weight ester group and a low molecular weight ester group, particularly in the ratio as stated above. Such combined presence is critical to the viscosity properties of the mixed ester, both from the standpoint of its viscosity modifying characteristics and from the standpoint of its thickening effect upon lubricating compositions in which it is used as an additive.

In reference to the size of the ester groups, it is pointed out that an ester radical is represented by the formula

-C(O)(OR)

and that the number of carbon atoms in an ester radical is the combined total of the carbon atoms of the carbonyl group and the carbon atoms of the ester group i.e., the (OR) group.

An optional element of this ester is the presence of a polyamino group derived from a particular amino compound, i.e., one in which there is one primary or secondary amino group and at least one mono-functional

amino group. Such polyamino groups, when present in this mixed ester in the proportion stated above enhances the dispersability of such esters in lubricant compositions and additive concentrates for lubricant compositions.

Still another essential element of the mixed ester is the extent of esterification in relation to the extent of neutralization of the unesterified carboxy groups of the carboxy-containing interpolymer through the conversion thereof to the optional polyamino-containing groups. For convenience, the relative proportions of the high molecular weight ester group to the low molecular weight ester group and to the polyamino group are expressed in terms of molar ratios of (50-100):(5-50):(0.1-15), respectively. The preferred ratio is (70-85):(15-30):(3-4). It should be noted that the linkage described as the carbonyl-polyamino group may be imide, amide, or amidine and inasmuch as any such linkage is contemplated within the present invention, the term "carbonyl polyamino" is thought to be a convenient, generic expression useful for the purpose of defining the inventive concept. In a particularly advantageous embodiment of the invention such linkage is imide or predominantly imide.

Still another important element of the mixed ester is the molecular weight of the carboxy-containing interpolymer. For convenience, the molecular weight is expressed in terms of the "reduced specific viscosity" of the interpolymer which is a widely recognized means of expressing the molecular size of a polymeric substance. As used herein, the reduced specific viscosity (abbreviated as RSV) is the value obtained in accordance with the formula

$$RSV = \frac{\text{Relative Viscosity} - 1}{\text{Concentration}}$$

wherein the relative viscosity is determined by measuring, by means of a dilution viscometer, the viscosity of a solution of one gram of the interpolymer in 10 ml. of acetone and the viscosity of acetone at  $30^\circ \pm 0.02^\circ \text{ C}$ . For purpose of computation by the above formula, the concentration is adjusted to 0.4 gram of the interpolymer per 100 ml. of acetone. A more detailed discussion of the reduced specific viscosity, also known as the specific viscosity, as well as its relationship to the average molecular weight of an interpolymer, appears in Paul J. Flory, *Principles of Polymer Chemistry*, (1953 Edition) pages 308 et seq.

While interpolymers having reduced specific viscosity of from about 0.05 to about 2 are contemplated in the mixed ester, the preferred interpolymers are those having a reduced specific viscosity of from about 0.1 to about 1. In most instances, interpolymers having a reduced specific viscosity of from about 0.1 to about 0.8 are particularly preferred.

From the standpoint of utility, as well as for commercial and economical reasons, esters in which the high molecular weight ester group has from 8 to 24 aliphatic carbon atoms, the low molecular weight ester group has from 3 to 5 carbon atoms, and the carbonyl amino group is derived from a primary-aminoalkyl-substituted tertiary amine, particularly heterocyclic amines, are preferred. Specific examples of the high molecular weight carboxylic ester group, i.e., the (OR) group of the ester radical (i.e.,  $-(\text{O})(\text{OR})$ ) include heptyloxy, isoctyloxy, decyloxy, dodecyloxy, tridecyloxy, tetradecyloxy, pentadecyloxy, octadecyloxy, eicosyloxy, tricosyloxy, tetracosyloxy, etc. Specific examples of

low molecular weight groups include methoxy, ethoxy, n-propoxy, isopropoxy, n-butyloxy, sec-butyloxy, iso-butyloxy, n-pentyloxy, neo-pentyloxy, n-hexyloxy, cyclohexyloxy, xyloxyloxy, 2-methyl-buty-1-oxy, 2,3-dimethyl-buty-1-oxy, etc. In most instances, alkoxy groups of suitable size comprise the preferred high and low molecular weight ester groups. Polar substituents may be present in such ester groups. Examples of polar substituents are chloro, bromo, ether, nitro, etc.

Examples of the carbonyl polyamino group include those derived from polyamino compounds having one primary or secondary amino group and at least one mono-functional amino group such as tertiary-amino or heterocyclic amino group. Such compounds may thus be tertiary-amino substituted primary or secondary amines or other substituted primary or secondary amines in which the substituent is derived from pyrroles, pyrrolidones, caprolactams, oxazolidones, oxazoles, thiazoles, pyrazoles, pyrazolines, imidazoles, imidazolines, thiazines, oxazines, diazines, oxycarbamyl, thiocarbamyl, uracils, hydantoins, thiohydantoins, guanidines, ureas, sulfonamides, phosphoramides, phenothiazines, amidines, etc. Examples of such polyamino compounds include dimethylamino-ethylamine, dibutylamino-ethylamine, 3-dimethylamino-1-propylamine, 4-methylethylamino-1-butylamine, pyridyl-ethylamine, N-morpholino-ethylamine, tetrahydropyridyl-ethylamine, bis-(dimethylamino)propyl-amine, bis(dieethylamino)ethylamine, N,N-dimethyl-p-phenylene diamine, piperidylethylamine, 1-aminoethyl pyrazole, 1-(methylamino)pyrazoline, 1-methyl-4-amino-octyl pyrazole, 1-aminoobutyl imidazole, 4-aminoethyl thiazole, 2-aminoethyl pyridine, ortho-amino-ethyl-N,N-dimethylbenzenesulfamide, N-aminoethyl phenothiazine, N-aminoethylacetamide, 1-aminophenyl-2-aminoethyl pyridine, N-methyl-N-aminoethyl-S-ethyl-dithiocarbamate, etc. Preferred polyamino compounds include the N-aminoalkyl-substituted morpholines such as aminopropyl morpholine. For the most part, the polyamino compounds are those which contain only one primary-amino or secondary-amino group and, preferably at least one tertiary-amino group. The tertiary amino group is preferably a heterocyclic amino group. In some instances polyamino compounds may contain up to about 6 amino groups although, in most instances, they contain one primary amino group and either one or two tertiary amino groups. The polyamino compounds may be aromatic or aliphatic amines and are preferably heterocyclic amines such as amino-alkyl-substituted morpholines, piperazines, pyridines, benzopyrroles, quinolines, pyrroles, etc. They are usually amines having from 4 to about 30 carbon atoms, preferably from 4 to about 12 carbon atoms. Polar substituents may likewise be present in the polyamines.

The carboxy-containing interpolymers include principally interpolymers of alpha, beta-unsaturated acids or anhydrides such as maleic anhydride or itaconic anhydride with olefins (aromatic or aliphatic) such as ethylene, propylene, isobutene or styrene, or substituted styrene wherein the substituent is a hydrocarbyl group containing from 1 up to about 18 carbon atoms. The styrene-maleic anhydride interpolymers are especially useful. They are obtained by polymerizing equal molar amounts of styrene and maleic anhydride, with or without one or more additional interpolymerizable comonomers. In lieu of styrene, an aliphatic olefin may be used,

such as ethylene, propylene or isobutene. In lieu of maleic anhydride, acrylic acid or methacrylic acid or ester thereof may be used. Such interpolymers are known in the art and need not be described in detail here. Where an interpolymerizable comonomer is contemplated, it should be present in a relatively minor proportion, i.e., less than about 0.3 mole, usually less than about 0.15 mole, per mole of either the olefin (e.g. styrene) or the alpha, beta-unsaturated acid or anhydride (e.g. maleic anhydride). Various methods of interpolymerizing styrene and maleic anhydride are known in the art and need not be discussed in detail here. For purpose of illustration, the interpolymerizable comonomers include the vinyl monomers such as vinyl acetate, acrylonitrile, methylacrylate, methylmethacrylate, acrylic acid, vinyl methyl ether, vinyl ethyl ether, vinyl chloride, isobutene or the like.

The nitrogen-containing esters of the mixed ester are most conveniently prepared by first 100 percent esterifying the carboxy-containing interpolymer with a relatively high molecular weight alcohol and a relatively low molecular weight alcohol. When the optional (C) is employed, the high molecular weight alcohol and low molecular weight alcohol are utilized to convert at least about 50% and no more than about 98% of the carboxy radicals of the interpolymer to ester radicals and then neutralizing the remaining carboxy radicals with a poly-amino compound such as described above. To incorporate the appropriate amounts of the two alcohol groups into the interpolymer, the ratio of the high molecular weight alcohol to the low molecular weight alcohol used in the process should be within the range of from about 2:1 to about 9:1 on a molar basis. In most instances the ratio is from about 2.5:1 to about 5:1. More than one high molecular weight alcohol or low molecular weight alcohol may be used in the process; so also may be used commercial alcohol mixtures such as the so-called Oxalcohols which comprise, for example mixtures of alcohols having from 8 to about 24 carbon atoms. A particularly useful class of alcohols are the commercial alcohols or alcohol mixtures comprising decylalcohol, dodecyl alcohol, tridecyl alcohol, tetradecyl alcohol, pentadecyl alcohol, hexadecyl alcohol, heptadecyl alcohol and octadecyl alcohol. Other alcohols useful in the process are illustrated by those which, upon esterification, yield the ester groups exemplified above.

The extent of esterification, as indicated previously, may range from about 50% to about 98% conversion of the carboxy radicals of the interpolymer to ester radicals. In a preferred embodiment, the degree of esterification ranges from about 75% to about 95%.

The esterification can be accomplished simply by heating the carboxy-containing interpolymer and the alcohol or alcohols under conditions typical for effecting esterification. Such conditions usually include, for example, a temperature of at least about 80° C., preferably from about 150° C. to about 350° C., provided that the temperature be below the decomposition point of the reaction mixture, and the removal of water of esterification as the reaction proceeds. Such conditions may optionally include the use of an excess of the alcohol reactant so as to facilitate esterification, the use of a solvent or diluent such as mineral oil, toluene, benzene, xylene or the like and a esterification catalyst such as toluene sulfonic acid, sulfuric acid, aluminum chloride, boron trifluoride-triethylamine, hydrochloric acid, ammonium sulfate, phosphoric acid, sodium methoxide or

the like. These conditions and variations thereof are well known in the art.

A particularly desirable method of effecting esterification involves first reacting the carboxy-containing interpolymer with the relatively high molecular weight alcohol and then reacting the partially esterified interpolymer with the relatively low molecular weight alcohol. A variation of this technique involves initiating the esterification with the relatively high molecular weight alcohol and before such esterification is complete, the relatively low molecular weight alcohol is introduced into the reaction mass so as to achieve a mixed esterification. In either event it has been discovered that a two-step esterification process whereby the carboxy-containing interpolymer is first esterified with the relatively high molecular weight alcohol so as to convert from about 50% to about 75% of the carboxy radicals to ester radicals and then with the relatively low molecular weight alcohol to achieve the finally desired degree of esterification results in products which have unusually beneficial viscosity properties.

The esterified interpolymer may optionally be treated with a polyamino compound in an amount so as to neutralize substantially all of the unesterified carboxy radicals of the interpolymer. The neutralization is preferably carried out at a temperature of at least about 80° C., often from about 120° C. to about 300° C., provided that the temperature does not exceed the decomposition point of the reaction mass. In most instances the neutralization temperature is between about 150° C. and 250° C. A slight excess of the stoichiometric amount of the amino compound is often desirable, so as to insure substantial completion of neutralization, i.e., no more than about 2% of the carboxy radicals initially present in the interpolymer remained unneutralized.

The following examples are illustrative of the preparation of the mixed ester of the present invention. Unless otherwise indicated all parts and percentages are by weight.

#### EXAMPLE C-1

A styrene-maleic interpolymer is obtained by preparing a solution of styrene (16.3 parts by weight) and maleic anhydride (12.9 parts) in a benzene-toluene solution (270 parts; weight ratio of benzene:toluene being 66.5:33.5) and contacting the solution at 86° C. in nitrogen atmosphere for 8 hours with a catalyst solution prepared by dissolving 70% benzoyl peroxide (0.42 part) in a similar benzene-toluene mixture (2.7 parts). The resulting product is a thick slurry of the interpolymer in the solvent mixture. To the slurry there is added mineral oil (141 parts) while the solvent mixture is being distilled off at 150° C. and then at 150° C. and 200 mm. Hg. To 209 parts of the stripped mineral oil-interpolymer slurry (the interpolymer having a reduced specific viscosity of 0.72) there are added toluene (25.2 parts), n-butyl alcohol (4.8 parts), a commercial alcohol consisting essentially of primary alcohols having from 12 to 18 carbon atoms (56.6 parts) and a commercial alcohol consisting of primary alcohols having from 8 to 10 carbon atoms (10 parts) and to the resulting mixture there is added 96% sulfuric acid (2.3 parts). The mixture is then heated at 150°-160° C. for 20 hours whereupon water is distilled off. An additional amount of sulfuric acid (0.18 part) together with an additional amount of n-butyl alcohol (3 parts) is added and the esterification is continued until 95% of the carboxy radicals of the polymer has been esterified. To the esterified interpoly-

mer, there is then added aminopropyl morpholine (3.71 parts; 10% in excess of the stoichiometric amount required to neutralize the remaining free carboxy radicals) and the resulting mixture is heated to 150°-160° C./10 mm. Hg to distill off toluene and any other volatile components. The stripped product is mixed with an additional amount of mineral oil (12 parts) filtered. The filtrate is a mineral oil solution of the nitrogen-containing mixed ester having a nitrogen content of 0.16-0.17%.

#### EXAMPLE C-2

The procedure of Example C-1 is followed except that the esterification is carried out in two steps, the first step being the esterification of the styrene-maleic interpolymer with the commercial alcohols having from 8 to 18 carbon atoms and the second step being the further esterification of the interpolymer with n-butyl alcohol.

#### EXAMPLE C-3

The procedure of Example C-1 is followed except that the esterification is carried out by first esterifying the styrene-maleic interpolymer with the commercial alcohol having from 8 to 18 carbon atoms until 70% of the carboxyl radicals of the interpolymer have been convened to ester radicals and thereupon continuing the esterification with any yet-unreacted commercial alcohols and n-butyl alcohol until 95% of the carbonyl radicals of the interpolymer have been convened to 30 ester radicals.

#### EXAMPLE C-4

The procedure of Example C-1 is followed except that the interpolymer is prepared by polymerizing a solution consisting of styrene (416 parts), maleic anhydride (392 parts), benzene (2153 parts) and toluene (5025 parts) in the presence of benzoyl peroxide (1.2 parts) at 65°-106° C. (The resulting interpolymer has a reduced specific viscosity of 0.45).

#### EXAMPLE C-5

The procedure of Example C-1 is followed except that the styrene-maleic anhydride is obtained by polymerizing a mixture of styrene (416 parts), maleic anhydride (392 parts), benzene (6101 parts) and toluene (2310 parts) in the presence of benzoyl peroxide (1.2 parts) at 78°-92° C. (The resulting interpolymer has a reduced specific viscosity of 0.91).

#### Example C-6

The procedure of Example C-1 is followed except that the styrene-maleic anhydride is prepared by the following procedure: Maleic anhydride (392 parts) is dissolved in benzene (6870 parts). To this mixture there is added styrene (416 parts) at 76° C. whereupon benzoyl peroxide (1.2 parts) is added. The polymerization mixture is maintained at 80°-82° C. for about 5 hours. (The resulting interpolymer has a reduced specific viscosity of 1.24.)

#### EXAMPLE C-7

The procedure of Example C-1 is followed except that acetone (1340 parts) is used in place of benzene as the polymerization solvent and that azobisisobutyronitrile (0.3 part) is used in place of benzoyl peroxide as a polymerization catalyst.

#### EXAMPLE C-8

An interpolymer (0.86 carboxyl equivalent) of styrene and maleic anhydride (prepared from an equal molar mixture of styrene and maleic anhydride and having a reduced specific viscosity of 0.69) is mixed with mineral oil to form a slurry, and then esterified with a commercial alcohol mixture (0.77 mole; comprising primary alcohols having from 8 to 18 carbon atoms) 5 at 150°-160° C. in the presence of a catalytic amount of sulfuric acid until about 70% of the carboxyl radicals are convened to ester radicals. The partially esterified interpolymer is then further esterified with a n-butyl alcohol (0.31 mole) until 95% of the carboxyl radicals of 10 the interpolymer are convened to the mixed ester radicals. The esterified interpolymer is then treated with aminopropyl morpholine (slight excess of the stoichiometric amount to neutralize the free carboxyl radicals of the interpolymer) at 150°-160° C. until the resulting 15 product is substantially neutral (acid number of 1 to phenolphthalein indicator). The resulting product is mixed with mineral oil so as to form an oil solution containing 34% of the polymeric product.

Examples C-1 through C-8 are prepared using mineral oil as the diluent. All of the mineral oil or a portion thereof may be replaced with the triglyceride oil (A). The preferred triglyceride oil is the high oleic sunflower oil.

#### EXAMPLE C-9

Charged to a 12 liter 4 neck flask is 3621 parts of the interpolymer of Example C-8 as a toluene slurry. The percent toluene is about 76 percent. Stirring is begun and 933 parts (4.3 equivalents) Alfol 1218 alcohol and 1370 parts xylene are added. The contents are heated and toluene is removed by distillation. Additional xylene is added in increments of 500, 500, 300 and 300 parts while continuing to remove toluene, the object being to replace the lower boiling toluene with the 20 higher boiling xylene. The removal of solvent is stopped when the temperature of 140° C. is reached. The flask is then fitted with an addition funnel and the condenser is set to reflux. At 140° C., 23.6 parts (0.17 equivalents) methanesulfonic acid in 432 parts (3 equivalents) Alfol 810 alcohol is added in about 20 minutes. The contents are stirred overnight at reflux while collecting water in a Dean Stark trap. Then added is 185 parts (2.5 equivalents) of n-butanol containing therein 3.0 parts (0.02 equivalents) of methanesulfonic acid. 25 This addition occurs over a 60 minute time period. The contents are maintained at reflux for 8 hours and then an additional 60 parts (0.8 equivalents) n-butanol is added and the contents are permitted to reflux overnight. At 142° C. is added 49.5 parts (0.34 equivalents) aminopropylmorpholine in 60 minutes. After a 2 hour reflux 30 13.6 parts (equivalents) 50% aqueous sodium hydroxide is added over 60 minutes and after an additional 60 minutes of stirring there is added 17 parts of an alkylated phenol.

To a 1 liter flask is added 495 parts of the above esterified product. The contents are heated to 140° C. and 337 parts Sunyl® 80 is added. Solvent is removed at 155° C. with nitrogen blowing at 1 cubic foot per hour. The final stripping conditions are 155° C. and 20 mm Hg. At 100° C. the contents are filtered using diatomaceous earth. The filtrate is a vegetable oil solution of the nitrogen-containing mixed ester having a nitrogen content of 0.14%.

Examples C-10 and C-11 employ an interpolymerizable monomer as part of the carboxy-containing interpolymer.

#### EXAMPLE C-10

One mole each of maleic anhydride and styrene and 0.05 moles methyl methacrylate are polymerized in toluene in the presence of benzoyl peroxide (1.5 parts) at 75°-95° C. The resulting interpolymer has a reduced specific viscosity of 0.13 and is a 12% slurry in toluene. Added to a 2 liter 4 neck flask is 868 parts (1 equivalent) of the polymer along with 68 parts (0.25 equivalents) oleyl alcohol, 55 parts (0.25 equivalents) Neodol 45, 55 parts (0.25 equivalents) Alfol 1218 and 36 parts (0.25 equivalents) Alfol 8-10. The contents are heated to 115° C. and added is 2 parts (0.02 moles) methanesulfonic acid. After a 2 hour reaction period, toluene is distilled off. With a neutralization number of 18.7 to phenolphthalein (indicating an 89% esterification), 15 parts (0.20 equivalents) n-butanol is added dropwise over 5 hours. The neutralization number/esterification level is 14.0/92.5%. Then added is 1.6 parts (0.02 moles) 50% aqueous sodium hydroxide to neutralize the catalyst. This is followed by the addition of 5.5 parts (0.038 equivalents) of aminopropylmorpholine and 400 parts Sunyl® 80. The contents are vacuum stripped to 15 millimeters mercury at 100° C. and filtered using a diatomaceous earth filter aid. The filtrate is the product containing 0.18 percent nitrogen and 54.9 percent Sunyl® 80.

The following example is similar to Example C-10 but employs different alcohols and different levels in a different order of addition.

#### EXAMPLE C-11

Added to a 2 liter 4 neck flask is 868 parts (1 equivalent) of the polymer of Example C-10, 9.25 parts (0.125 equivalents) isobutyl alcohol, 33.8 parts (0.125 equivalents) oleyl alcohol, 11 parts each (0.125 equivalents) of 2-methyl-1-butanol, 3-methyl-1-butanol and 1-pentanol, 23.4 parts (0.125 equivalents) hexyl alcohol, and 16.25 parts each (0.125 equivalents) 1-octanol and 2-octanol. At 110° C. 2 parts (0.02 moles) methanesulfonic acid is added. One hour later toluene is distilled off and when the distillation is complete, the neutralization number/esterification level is 62.5/70 percent. At 140° C. 31.2 parts (0.43 equivalents) n-butanol is added dropwise over 28 hours and the neutralization number/esterification level is 36.0/79.3 percent. At 120° C. 0.3 parts (0.03 moles) methanesulfonic acid is added followed by 20.4 parts (0.20 equivalents) hexyl alcohol. After esterification the neutralization number/esterification level is 10.5/95 percent. Then added is 1.9 parts (0.023 moles) of 50% sodium hydroxide followed by 5.9 parts (0.04 equivalents) aminopropylmorpholine and 400 parts Sunyl® 80. The contents are filtered and the product has a nitrogen analysis of 0.18 percent.

#### Acrylate Polymers

In another aspect Component (C) is at least one hydrocarbon-soluble acrylate polymer of the formula



wherein  $R^5$  is hydrogen or a lower alkyl group containing from 1 to about 4 carbon atoms,  $R^6$  is a mixture of

alkyl, cycloalkyl or aromatic groups containing from about 4 to about 24 carbon atoms, and  $x$  is an integer providing a weight average molecular weight (Mw) to the acrylate polymer of about 5000 to about 1,000,000.

Preferably  $R^5$  is a methyl or ethyl group and more preferably, a methyl group.  $R^6$  is primarily a mixture of alkyl groups containing from 4 to about 18 carbon atoms. In one embodiment, the weight average molecular weight of the acrylate polymer is from about 100,000 to about 1,000,000 and in other embodiments, the molecular weight of the polymer may be from 100,000 to about 700,000 and 300,000 to about 700,000.

Specific examples of the alkyl groups  $R^6$  which may be included in the polymers of the present invention include, for example, n-butyl, octyl, decyl, dodecyl, tridecyl, octadecyl, hexadecyl, octadecyl. The mixture of alkyl groups can be varied so long as the resulting polymer is hydrocarbon-soluble.

The following examples are illustrative of the preparations of the acrylate polymers of the present invention. All parts and percentages are by weight unless indicated to the contrary.

#### EXAMPLE C-12

Added to a 2 liter 4 neck flask is 50.8 parts (0.20 moles) lauryl methacrylate, 44.4 parts (0.20) isobornyl methacrylate, 38.4 parts (0.20 moles) 2-phenoxy ethyl acrylate, 37.6 parts (0.20 moles) 2-ethylhexyl acrylate, 45.2 parts (0.20 moles) isodecyl methacrylate and 500 parts toluene. At 100° C. 1 parts Vazo® 67 (2,2'azobis(2-methylbutyronitrile)) in 20 parts toluene is added over 7 hours. The reaction is held at 100° C. for 16 hours after which the temperature is increased to 120° C. to remove toluene and added is 216 parts of Sunyl® 80. Volatiles are removed by vacuum distillation at 20 millimeters mercury at 140° C. The contents are filtered to give the desired product.

#### EXAMPLE C-13

Added to a 2 liter 4 neck flask is 38.1 parts (0.15 moles) lauryl methacrylate, 48.6 parts (0.15 moles) stearyl acrylate, 28.2 parts (0.15 moles) 2-ethylhexyl methacrylate, 25.5 parts (0.15 moles) tetrahydrofurfuryl methacrylate, 33.9 parts (0.15 moles) isodecyl methacrylate and 500 parts toluene. At 100° C. 1 part Vazo® 67 in 20 parts toluene is added dropwise in 6 hours. After the addition is complete, the reaction mixture is held at 100° C. for 15.5 hours, toluene is distilled out and 174 parts Sunyl® 80 is added. The contents are vacuum stripped at 140° C. at 20 millimeters of mercury and filtered to give the desired product.

An example of a commercially available methacrylate ester polymer which has been found to be useful in the present invention is sold under the tradename of "Acryloid 702" by Rohm and Haas, wherein  $R^5$  is predominantly a mixture of n-butyl, tridecyl, and octadecyl groups. The weight average molecular weight (Mw) of the polymer is about 404,000 and the number average molecular weight (Mn) is about 118,000. Another commercially available methacrylate polymer useful in the present invention is available under the tradename of "Acryloid 954" by Rohm and Haas, wherein  $R^5$  is predominantly a mixture of n-butyl, decyl, tridecyl, octadecyl, and tetradecyl groups. The weight average molecular weight of Acryloid 954 is found to be about 440,000 and the number average molecular weight is about 111,000. Each of these commercially available

methacrylate polymers is sold in the form of a concentrate of about 40% by weight of the polymer in a light-colored mineral lubricating oil base. When the polymer is identified by the tradename, the amount of material added is intended to represent an amount of the commercially available Acryloid material including the oil.

Other commercially available polymethacrylates are available from Rohm and Haas Company as Acryloid 1253, Acryloid 1265, Acryloid 1263, Acryloid 1267, from Rohm GmbH as Viscoplex 0-410, Viscoplex 10-930, Viscoplex 5029, from Societe Francaise D'Organic-Synthese as Garbacryl T-84, Garbacryl T-78S, from Texaco as TLA 233, TLA 5010 and TC 10124. Some of these polymethacrylates may be PMA/OCP (olefin copolymer) type polymers.

#### Nitrogen-Containing Polyacrylate

Component (C) may also be a nitrogen-containing polymer prepared by polymerizing an acrylate ester monomer of the formula



wherein  $\text{R}^9$  is hydrogen or an alkyl group containing from 1 to about 4 carbon atoms and  $\text{R}^{10}$  is an alkyl, cycloalkyl or aromatic group containing from 4 to about 24 carbon atoms with a nitrogen containing monomer. For each mole of the acrylate ester monomer from 0.001-1.0 moles of the nitrogen containing monomer is employed. The reaction is carried out at a temperature of from 50° C. up to about 250° C. Non-limiting examples of nitrogen containing monomers are 4-vinylpyridine, 2-vinylpyridine, 2-n-morpholinoethyl acrylate, N,N-dimethylaminoethyl acrylate, and N,N-dimethylaminopropyl methacrylate.

The following example is illustrative of the preparation of the nitrogen-containing polyacrylate. All parts and percentages are by weight unless indicated otherwise.

#### EXAMPLE C-14

Added to a 2 liter 4 neck flask is 50.8 parts (0.2 moles) lauryl methacrylate, 44.4 parts (0.20 moles) isobornyl methacrylate, 38.4 parts (0.20 moles) 2-phenoxyethyl acrylate, 37.6 parts (0.20 moles) 2-ethylhexyl acrylate, 45.2 parts (0.20 moles) isodecyl methacrylate, 21 parts (0.20 moles) 4-vinylpyridine and 500 parts toluene. At 100° C. 1 part Vazo 67 in 20 parts toluene is added dropwise in 8 hours. After maintaining the temperature at 100° C. for an additional 20 hours, an additional 0.5 parts Vazo 67 in 10 parts toluene is added in 3 hours. Toluene is then removed by distillation, 235 parts Suyl (R) 80 is added and the contents are vacuum stripped to 25 millimeters mercury at 140° C. The contents are filtered to give a product with 0.71 percent nitrogen.

A few companies that make nitrogen-containing polyacrylates are Rohm and Haas, Rohm GmbH, Texaco, Albright & Wilson, Societe Francaise and D'Organic-Synthese (SFOS).

#### Methylene Linked Aromatic Compounds

Another PPD having utility in this invention is a mixture of compounds having the general structural formula:



wherein the Ar, Ar' and Ar'' are independently an aromatic moiety and each aromatic moiety is substituted

with 0 to 3 substituents (the preferred aromatic precursor being naphthalene),  $\text{R}^7$  and  $\text{R}^8$  are independently straight or branch chain alkynes containing 1 to 100 carbon atoms and  $n$  is 0 to 1000. U.S. Pat. No. 4,753,745 is incorporated herein by reference for its disclosure of methylene linked aromatic compounds.

#### EXAMPLE C-15

Naphthalene is mixed with seven parts of  $\text{CH}_2\text{Cl}_{12}$  and 0.2 parts of  $\text{AlCl}_3$ . Chlorinated hydrocarbon (2.7 parts) is added slowly into the reaction mixture at 15° C. The reaction mixture is held for 5 hours at ambient temperature or until the release of  $\text{HCl}$  is complete. The mixture is then cooled to about 5° C. and 7.3 parts of an alpha olefin mixture is added over 2 hours while maintaining the temperature of the reaction mixture between 0° and 10° C.

The catalyst is decomposed by the careful addition of 0.8 parts 50% aqueous  $\text{NaOH}$ . The aqueous layer is separated and the organic layer is purged with  $\text{N}_2$  and heated to 140° C. and 3 mm Hg to remove the volatiles. The residue is filtered to yield 97% of the theoretical yield weight of the product.

#### (D) The Performance Additive

In addition to components (A), (B) and (C), the compositions of this invention also include (D), a performance additive. The performance enhanced by these additives in the areas of anti-wear, oxidation inhibition, rust/corrosion inhibition, metal passivation, extreme pressure, friction modification, viscosity modification, foam inhibition, emulsification, demulsification, lubricity, dispersancy and detergency and the like.

The performance additive (D) is selected from the group consisting of

- (1) an alkyl phenol,
- (2) a benzotriazole,
- (3) a phosphatide,
- (4) a thiocarbamate,
- (5) citric acid or its derivative,
- (6) a coupled phosphorus-containing amide, or
- (7) a methylacrylate derivative
- (8) a metal overbased composition,
- (9) a carboxylic dispersant
- (10) a nitrogen-containing organic composition,
- (11) a zinc salt,
- (12) a sulfurized composition,
- (13) a viscosity index improver, and
- (14) an aromatic amine.

#### (D)(1) The Alkyl Phenol

Component (D-1) is an alkyl phenol of the formula



wherein  $\text{R}^{11}$  is an alkyl group containing from 1 up to about 24 carbon atoms and  $a$  is an integer of from 1 up to 5. Preferably  $\text{R}^{11}$  contains from 4 to 18 carbon atoms and most preferably from 4 to 12 carbon atoms.  $\text{R}^{11}$  may be either straight chained or branched chained and branched chained is preferred. The preferred value for  $a$  is an integer of from 1 to 4 and most preferred is from

1 to 3. An especially preferred value for  $a$  is 2. When  $a$  is not 5, it is preferred that the position para to the OH group be open.

Mixtures of alkyl phenols may be employed. Preferably the phenol is a butyl substituted phenol containing 2 or 3 t-butyl groups. When  $a$  is 2, the t-butyl groups occupy the 2,6-position, that is, the phenol is sterically hindered:



When  $a$  is 3, the t-butyl groups occupy the 2,4,6-position.

(D)(2) The Benzotriazole

The benzotriazole compound is of the formula



wherein  $R^{12}$  is hydrogen a straight or branched-chain alkyl group containing from 1 up to about 24 carbon atoms, preferably 1 to 12 carbon atoms and most preferably 1 carbon atom. When  $R^{12}$  is 1 carbon atom the benzotriazole compound is tolyltriazole of the formula



Tolyltriazole is available under the trade name Cobratrac TT-100 from Sherwin-Williams Chemical.

(D)(3) The Phosphatide

Another metal deactivator are the phosphatides of the formula



wherein  $R^{13}$  and  $R^{14}$  are aliphatic hydrocarbyl groups containing from 8 to about 24 carbon atoms and  $G$  is selected from the group consisting of hydrogen,



such that the phosphatide is lecithin. Particularly effective phosphatides are soybean lecithin, corn lecithin,

peanut lecithin, sunflower lecithin, safflower lecithin and rapeseed lecithin.

(D)(4) The Thiocarbamate

The thiocarbamates are of the formula



10 wherein  $R^{15}$  is an alkyl group containing from 1 to about 24 carbon atoms, phenyl or alkyl phenyl wherein the alkyl group contains from 1 to about 18 carbon atoms. Preferably  $R^{15}$  is an alkyl group containing from 1 to 6 carbon atoms. The groups  $R^{16}$  and  $R^{17}$  are hydrogen or an alkyl group containing from 1 to about 6 carbon atoms, with the proviso that  $R^{16}$  and  $R^{17}$  are not both hydrogen.

(D)(5) The Citric Acid and its Derivatives

The citric acid or derivatives of citric acid are of the formula



30 wherein  $R^{18}$ ,  $R^{19}$  and  $R^{20}$  are independently hydrogen or aliphatic hydrocarbyl groups containing from 1 to about 12 carbon atoms, with the proviso that at least one of  $R^{18}$ ,  $R^{19}$  and  $R^{20}$  is an aliphatic hydrocarbyl group and preferably contains from 1 to about 6 carbon atoms.

(D)(6) The Coupled Phosphorus-Containing Amide

The coupled phosphorus-containing amide is a statistical mixture of compounds having the following formula



Considering  $X^1$  and  $X^2$ , it independently is oxygen or sulfur and preferably is sulfur whereas  $X^3$  is oxygen or 50 sulfur and preferably oxygen.  $R^{21}$  and  $R^{22}$  each independently is a hydrocarbyl, a hydrocarbyl-based thio or preferably a hydrocarbyl-based oxy group wherein the hydrocarbyl portion contains 6 to 22 carbon atoms. The hydrocarbyl portion of  $R^{21}$  and  $R^{22}$  generally contains 55 from 1 to about 34 carbon atoms. When  $R^{27}$  is hydrogen and  $R^{28}$  is methylene,  $R^{21}$  and  $R^{22}$  will contain 6 to 12 carbon atoms in order to provide for sufficient oil solubility. The hydrocarbyl portion of  $R^{21}$  and  $R^{22}$  independently can be alkyl or aromatic. Although the hydrocarbyl portion of both  $R^{21}$  and  $R^{22}$  can be the same type of hydrocarbyl group, that is both alkyl or both aromatic, often one such group can be alkyl and the remaining group can be aromatic. Different coupled phosphorus-containing amide compounds which are 60 made by reacting a mixture of two or more different reactants each containing an alkyl hydrocarbyl group as well as an aromatic hydrocarbyl ( $R^{21}$  and  $R^{22}$ ) group herein. The same or different compounds are coupled 65

via different coupling groups  $R^{28}$  to form a statistical mixture of coupled compounds or are reacted with different compounds to provide different functional groups  $R^{28}$  thereon. U.S. Pat. No. 4,938,884 is incorporated herein by reference for its disclosure of coupled phosphorus containing amide.

A particularly preferred embodiment of (D)(6) includes a statistical mixture (i.e., coupled and uncoupled compounds each with different substituent groups providing a variety of different compounds) of different phosphorus containing amide compounds bonded to or couple by different  $R^{28}$  groups with the proviso that in general coupled phosphorus-containing amide the mixture includes some compounds wherein  $n'$  is 1 and  $R^{28}$  is  $-\text{CH}_2\text{OH}$  and also where  $n'$  is 2,  $R^{28}$  is



Any such statistical mixture is likely to include some coupled amide compounds of coupled phosphorus-containing amide wherein  $R^{28}$  is methylene. When  $R^{28}$  is methylene,  $R^{21}$  and  $R^{22}$  generally must contain more than 6 carbon atoms in order to maintain good oil solubility. When  $n'$  is 1,  $R^{25}$  is selected from the group consisting of H,  $-\text{ROH}$ ,  $-\text{ROR}$ ,  $-\text{RSR}$  and  $\text{RN}(\text{R})_2$  and when  $n'$  is 2 or 3,  $R^{28}$  is selected from the group consisting of



and when  $n'$  is 3,  $R^{27}$  is



wherein R is independently hydrogen or an alkyl moiety, alkylene or alkylidene of 1 to 12 carbon atoms and R' is hydrogen or an alkyl or carboxy alkyl moiety, alkylene or alkylidene of containing 1 to 60 carbon atoms, R is preferably methylene and R' is preferably an alkyl moiety of 1 to 28 carbons. When R and R' are linking groups, they may be alkylene and/or alkylidene, i.e., the linkage may be vicinal and/or geminal.

The following illustrate the preparation of the coupled phosphorus-containing compounds. All parts and percentages are by weight unless otherwise indicated.

#### EXAMPLE (D)(6)-1

To a mixture of 1775 parts (4.26 equivalents) of O,O-di-isoctyl phosphorodithioic acid and 980 parts of toluene under a nitrogen atmosphere are added 302 parts (4.26 equivalents) of acrylamide. The reaction mixture exotherms to about 56° C. and 77 parts (2.33 equivalents) of paraformaldehyde and 215 parts (0.11 equivalent) of p-toluenesulfonic acid hydrate are added. Heating is continued at reflux (92°-127° C.) while removing 48 parts of water. Upon cooling the mixture to 100° C., 9.2 parts (0.11 equivalent) of sodium bicarbonate is added and cooling continued to about 30° C. A

vacuum is applied (15 mm. Hg) and toluene solvent removed while raising the temperature to 110° C. The residue is filtered through a filter aid and the filtrate is the desired product. The product contains 6.86% P (6.74% theory).

#### EXAMPLE (D)(6)-2

To a mixture of 1494 parts (3.79 equivalents) of O,O-di-isoctyl phosphorodithioic acid and 800 parts of toluene under a nitrogen atmosphere are added 537 parts (3.79 equivalents) of 50% aqueous acrylamide solution over a period of one hour. The reaction mixture exotherms to about 53° C. and 64 parts (1.93 equivalents) of paraformaldehyde and 18 parts (0.095 equivalent) of p-toluenesulfonic acid hydrate are added. Heating is continued at reflux (91°-126° C.) for 4 hours while collecting 305 parts of water. The mixture is cooled to about 90° C. and 7.6 parts (0.095 equivalent) of 50% aqueous sodium hydroxide solution are added. Cooling is continued to about 30° C. and a vacuum is applied (15 mm Hg). Toluene solvent is removed while raising the temperature to 110° C. The residue is filtered through a filter aid and the filtrate is the desired product. The product contains 6.90% P (6.75% theory) and 2.92% N (2.97% theory).

#### (D)(7) The Methylacrylate Derivative

The methylacrylate derivative is formed by the reaction of equal molar mounts of a phosphorus acid of the formula



with methylacrylate wherein  $\text{X}^1$  and  $\text{X}^2$  are as defined above in (D)(6) and  $\text{R}^{29}$  and  $\text{R}^{30}$  are each independently a hydrocarbyl, a hydrocarbyl-based thio or preferably a hydrocarbyl-based oxy group wherein the hydrocarbyl portion contains from 1 to about 30 carbon atoms. Preferably  $\text{R}^{29}$  and  $\text{R}^{30}$  are hydrocarbyl-based oxy groups wherein the hydrocarbyl group contains from 1 to 12 carbon atoms and  $\text{X}^1$  and  $\text{X}^2$  are sulfur. Since the reaction does not go to completion, the remaining acidity is neutralized with propylene oxide.

In preparing (D)(7), methylacrylate is added to the phosphorus acid and at the end of this addition, propylene oxide is added. Generally one mole of propylene oxide is employed for every 20-25 moles of phosphorus acid.

The following illustrates the preparation of the methylacrylate derivative. All parts and percentages are by weight unless otherwise indicated.

#### EXAMPLE (D)(7)-1

To 2652 parts (9.04 equivalents) of a O,O-di-alkyl phosphorodithioic acid prepared from a mixture of 65 mole percent iso-butyl alcohol and 35 mole percent iso-amyl alcohol is added 776 parts (9.04 equivalents) of methyl acrylate. The methyl acrylate addition is done dropwise and the temperature increases from 60° to 93° C. The contents are held at this temperature for 6 hours and then cooled to 35° C. at which 23 parts (0.04 equivalents) propylene oxide is added dropwise. The contents are filtered to give a product having a % phosphorus of 7.54 (8.12% theory).

#### (D)(8) The Metal Overbased Composition

Overbased salts of organic acids are widely known to those of ordinary skill in the art and generally include metal salts wherein the amount of metal present in them exceeds the stoichiometric amount. Such salts are said to have conversion levels in excess of 100% (i.e., they comprise more than 100% of the theoretical amount of metal needed to convert the acid to its "normal" "neutral" salt). Such salts are often said to have metal ratios in excess of one (i.e., the ratio of equivalents of metal to equivalents of organic acid present in the salt is greater than that required to provide the normal or neutral salt which required only a stoichiometric ratio of 1:1). They are commonly referred to as overbased, hyperbased or superbased salts and are usually salts of organic sulfur acids, organic phosphorus acids, carboxylic acids, phenols or mixtures of two or more of any of these. As a skilled worker would realize, mixtures of such overbased salts can also be used.

The terminology "metal ratio" is used in the prior art and herein to designate the ratio of the total chemical equivalents of the metal in the overbased salt to the chemical equivalents of the metal in the salt which would be expected to result in the reaction between the organic acid to be overbased and the basically reacting metal compound according to the known chemical reactivity and stoichiometry of the two reactants. Thus, in a normal or neutral salt the metal ratio is one and in an overbased salt the metal ratio is greater than one.

The overbased salts used as (D)(8) in this invention usually have metal ratios of at least about 3:1. Typically, they have ratios of at least about 12:1. Usually they have metal ratios not exceeding about 40:1. Typically salts having ratios of about 12:1 to about 20:1 are used.

The basically reacting metal compounds used to make these overbased salts are usually an alkali or alkaline earth metal compound (i.e., the Group IA, IIA, and IIB metals excluding francium and radium and typically excluding rubidium, cesium and beryllium) although other basically reacting metal compounds can be used. Compounds of Ca, Ba, Mg, Na and Li, such as their hydroxides and alkoxides of lower alkanols are usually used as basic metal compounds in preparing these overbased salts but others can be used as shown by the prior art incorporated by reference herein. Overbased salts containing a mixture of ions of two or more of these metals can be used in the present invention.

These overbased salts can be of oil-soluble organic sulfur acids such as sulfonic, sulfamic, thiosulfonic, sulfinic, sulfonic, partial ester sulfuric, sulfurous and thiosulfuric acid. Generally they are salts of carbocyclic or aliphatic sulfonic acids.

The carboxylic sulfonic acids include the mono- or poly-nuclear aromatic or cycloaliphatic compounds. The oil-soluble sulfonates can be represented for the most part by the following formulae:



In the above formulae, M is either a metal cation as described hereinabove or hydrogen; T is a cyclic nucleus such as, for example, benzene, naphthalene, anthracene, phenanthrene, diphenylene oxide, thianthrene, phenothioxine, diphenylene sulfide, phenothiazine, diphenyl oxide, diphenyl sulfide, diphenylamine, cyclohexane, petroleum naphthenes, decahydro-naphthalene, cyclopentane, etc.: R in Formula I is an aliphatic group such as alkyl, alkenyl, alkoxy, alkoxyalkyl,

carboalkoxyalkyl and contains at least about 15 carbon atoms, R<sup>31</sup> in Formula II is an aliphatic radical containing at least about 15 carbon atoms and M is either a metal cation or hydrogen. Examples of type of the R<sup>31</sup> radical are alkyl, alkenyl, alkoxyalkyl, carboalkoxyalkyl, etc. Specific examples of R<sup>31</sup> are groups derived from petrolatum, saturated and unsaturated paraffin wax, and polyolefins, including polymerized C<sub>2</sub>, C<sub>3</sub>, C<sub>4</sub>, C<sub>5</sub>, C<sub>6</sub>, etc., olefins containing from about 15 to 7000 or more carbon atoms. The groups T, R, and R<sup>31</sup> in the above formulae can also contain other inorganic or organic substituents in addition to those enumerated above such as, for example, hydroxy, mercapto, halogen, nitro, amino, nitroso, sulfide, disulfide, etc. In Formula I, x, y, z and b are at least 1, and likewise in Formula II, a, b and d are at least 1.

Specific examples of sulfonic acids useful in this invention are mahogany sulfonic acids; bright stock sulfonic acids; sulfonic acids derived from lubricating oil fractions having a Saybolt viscosity from about 100 seconds at 100° F. to about 200 seconds at 210° F; petrolatum sulfonic acids; mono- and poly-wax substituted sulfonic and polysulfonic acids of, e.g., benzene, naphthalene, phenol, diphenyl ether, naphthalene disulfide, diphenylamine, thiophene, alpha-chloronaphthalene, etc.; other substituted sulfonic acids such as alkyl benzene sulfonic acids (where the alkyl group has at least 8 carbons), cetylphenol mono-sulfide sulfonic acids, dicetyl thianthrene disulfonic acids, dilauryl beta naphthyl sulfonic acid, dicapryl nitronaphthalene sulfonic acids, and alkaryl sulfonic acids such as dodecyl benzene "bottoms" sulfonic acids.

The latter acids derived from benzene which has been alkylated with propylene tetramers or isobutene trimers to introduce 1,2,3, or more branched-chain C<sub>12</sub> substituents on the benzene ring. Dodecyl benzene bottoms, principally mixtures of mono-and di-dodecyl benzenes, are available as by-products from the manufacture of household detergents. Similar products obtained from alkylation bottoms formed during manufacture of linear alkyl sulfonates (LAS) are also useful in making the sulfonates used in this invention.

The production of sulfonates from detergent manufacture-by-products by reaction with, e.g., SO<sub>3</sub>, is well known to those skilled in the art. See, for example, the article "Sulfonates" in Kirk-Othmer "Encyclopedia of Chemical Technology", Second Edition, Vol. 19, pp. 291 at seq. published by John Wiley & Sons, New York (1969).

Other descriptions of overbased sulfonate salts and techniques for making them can be found in the following U.S. Pat. Nos. 2,174,110; 2,174,506; 2,174,508; 2,193,824; 2,197,800; 2,202,781; 2,212,786; 2,213,360; 2,228,598; 2,223,676; 2,239,974; 2,263,312; 2,276,090; 2,276,297; 2,315,514; 2,319,121; 2,321,022; 2,333,568; 2,333,788; 2,335,259; 2,337,552; 2,346,568; 2,366,027; 2,374,193; 2,383,319; 3,312,618; 3,471,403; 3,488,284; 3,595,790; and 3,798,012. These are hereby incorporated by reference for their disclosures in this regard.

Also included are aliphatic sulfonic acids such as paraffin wax sulfonic acids, unsaturated paraffin wax sulfonic acids, hydroxy-substituted paraffin wax sulfonic acids, hexapropylene sulfonic acids, tetra-amylene sulfonic acids, polyisobutene sulfonic acids wherein the polyisobutene contains from 20 to 7000 or more carbon atoms, chloro-substituted paraffin wax sulfonic acids, nitroparaffin wax sulfonic acids, etc.; cycloaliphatic

sulfonic acids such as petroleum naphthalene sulfonic acids, cetyl cyclopentyl sulfonic acids, lauryl cyclohexyl sulfonic acids, bis-(di-isobutyl) cyclohexyl sulfonic acids, etc.

With respect to the sulfonic acids or salts thereof described herein and in the appended claims, it is intended that the term "petroleum sulfonic acids" or "petroleum sulfonates" includes all sulfonic acids or the salts thereof derived from petroleum products. A particularly valuable group of petroleum sulfonic acids are the mahogany sulfonic acids (so called because of their reddish-brown color) obtained as a by-product from the manufacture of petroleum white oils by a sulfuric acid process.

Generally Group IA, IIA and IIB overbased salts of the above-described synthetic and petroleum sulfonic acids are typically useful in making (D)(8) of this invention.

The carboxylic acids from which suitable overbased salts for use in this invention can be made include aliphatic, cycloaliphatic, and aromatic mono- and polybasic carboxylic acids such as the naphthenic acids, alkyl- or alkenyl-substituted cyclopentanoic acids, alkyl- or alkenyl-substituted cyclohexanoic acids, alkyl- or alkenyl-substituted aromatic carboxylic acids. The aliphatic acids generally contain at least 8 carbon atoms and preferably at least 12 carbon atoms. Usually they have no more than about 400 carbon atoms. Generally, if the aliphatic carbon chain is branched, the acids are more oil-soluble for any given carbon atoms content. The cycloaliphatic and aliphatic carboxylic acids can be saturated or unsaturated. Specific examples include 2-ethylhexanoic acid, a-linolenic acid, propylene-tetramer-substituted maleic acid, behenic acid, isostearic acid, pelargonic acid, capric acid, palmitoleic acid, linoleic acid, lauric acid, oleic acid, ricinoleic acid, undecylic acid, diocetyl-cyclopentane carboxylic acid, myristic acid, dilauryldecahydronaphthalene carboxylic acid, stearyl-octahydroindene carboxylic acid, palmitic acid, commercially available mixtures of two or more carboxylic acids such as tall oil acids, rosin acids, and the like.

A typical group of oil-soluble carboxylic acids useful in preparing the salts used in the present invention are the oil-soluble aromatic carboxylic acids. These acids are represented by the general formula:



(III)

wherein  $R^*$  is an aliphatic hydrocarbon-based group of at least 4 carbon atoms, and no more than about 400 aliphatic carbon atoms,  $g$  is an integer from one to four,  $AR^*$  is a polyvalent aromatic hydrocarbon nucleus of up to about 14 carbon atoms, each  $X$  is independently a sulfur or oxygen atom, and  $f$  is an integer of from one to four with the proviso that  $R^*$  and  $g$  are such that there is an average of at least 8 aliphatic carbon atoms provided by the  $R^*$  groups for each acid molecule represented by Formula III. Examples of aromatic nuclei represented by the variable  $AR^*$  are the polyvalent aromatic radicals derived from benzene, naphthalene, anthracene, phenanthrene, indene, fluorene, biphenyl, and the like. Generally, the radical represented by  $AR^*$  will be a polyvalent nucleus derived from benzene or naphthalene such as phenylenes and naphthylene, e.g., methylenes, ethoxyphenylenes, nitrophenylenes,

isopropylenes, hydroxyphenylenes, mercaptophenylenes, N,N-diethylaminophenylenes, chlorophenylenes, N,N-diethylaminophenylenes, chlorophenylenes, di-propoxynaphthylenes, triethylnaphthylenes, and similar tri-, tetra-, pentavalent nuclei thereof, etc.

The  $R^*$  groups are usually hydrocarbyl groups, preferably groups such as alkyl or alkenyl radicals. However, the  $R^*$  groups can contain small number substituents such as phenyl, cycloalkyl (e.g., cyclohexyl, cyclopentyl, etc.) and nonhydrocarbon groups such as nitro, amino, halo (e.g., chloro, bromo, etc.), lower alkoxy, lower alkyl mercapto, oxo substituents (i.e.,  $=O$ ), thio groups (i.e.,  $=S$ ), interrupting groups such as  $-NH-$ ,  $-O-$ ,  $-S-$ , and the like provided the essentially hydrocarbon character of the  $R^*$  group is retained. The hydrocarbon character is retained for purposes of this invention so long as any non-carbon atoms present in the  $R^*$  groups do not account for more than about 10% of the total weight of the  $R^*$  groups.

Examples of  $R^*$  groups include butyl, isobutyl, pentyl, octyl, nonyl, dodecyl, docosyl, tetracontyl, 5-chlorohexyl, 4-ethoxypentyl, 4-hexenyl, 3-cyclohexyl-octyl, 4-(p-chlorophenyl)-octyl, 2,3,5-trimethylheptyl, 4-ethyl-5-methyloctyl, and substituents derived from polymerized olefins such as polychloroprenes, polyethylenes, polypropylenes, polyisobutylenes, ethylene-propylene copolymers, chlorinated olefin polymers, oxidized ethylene-propylene copolymers, and the like. Likewise, the group  $Ar^*$  may contain non-hydrocarbon substituents, for example, such diverse substituents as lower alkoxy, lower alkyl mercapto, nitro, halo, alkyl or alkenyl groups of less than 4 carbon atoms, hydroxy, mercapto, and the like.

Another group of useful carboxylic acids are those of the formula:



wherein  $R^*$ ,  $X$ ,  $Ar^*$ ,  $f$  and  $g$  are as defined in Formula III and  $p^*$  is an integer of 1 to 4, usually 1 or 2. Within this group, an especially preferred class of oil-soluble carboxylic acids are those of the formula:



wherein  $R^{**}$  in Formula V is an aliphatic hydrocarbon group containing at least 4 to about 400 carbon atoms,  $a^*$  is an integer of from 1 to 3,  $b^*$  is 1 or 2,  $c^*$  is zero, 1, or 2 and preferably 1 with the proviso that  $R^{**}$  and  $a^*$  are such that the acid molecules contain at least an average of about 12 aliphatic carbon atoms in the aliphatic hydrocarbon substituents per acid molecule. And within this latter group of oil-soluble carboxylic acids, the aliphatic-hydrocarbon substituted salicyclic acids

wherein each aliphatic hydrocarbon substituent contains an average of at least about 16 carbon atoms per substituent and 1 to 3 substituents per molecule are particularly useful. Salts prepared from such salicyclic acids wherein the aliphatic hydrocarbon substituents are derived from polymerized olefins, particularly polymerized lower 1-mono-olefins such as polyethylene, polypropylene, polyisobutylene, ethylene/propylene copolymers and the like and having average carbon contents of about 30 to about 400 carbon atoms.

The carboxylic acids corresponding to Formulae IV-V above are well known or can be prepared according to procedures known in the art. Carboxylic acids of the type illustrated by the above formulae and processes for preparing their overbased metal salts are well known and disclosed, for example, in such U.S. Pat. Nos. as 2,197,832; 2,197,835; 2,252,662; 2,252,664; 2,714,092; 3,410,798 and 3,595,791 which are incorporated by reference herein for their disclosures of acids and methods of preparing overbased salts.

Another type of overbased carboxylate salt used in making (D-3) of this invention are those derived from alkenyl succinates of the general formula:



(VI) 25

wherein  $R^*$  is as defined above in Formula IV. Such salts and means for making them are set forth in U. S. Pat. Nos. 3,271,130, 3,567,637 and 3,632,510, which are hereby incorporated by reference in this regard.

Other patents specifically describing techniques for making overbased salts of the hereinabove-described sulfonic acids, carboxylic acids, and mixtures of any two or more of these include U.S. Pat. Nos. 2,501,731; 2,616,904; 2,616,905; 2,616,906; 2,616,911; 2,616,924; 2,616,925; 2,617,049; 2,777,874; 3,027,325; 3,256,186; 3,282,835; 3,384,585; 3,373,108; 3,365,296; 3,342,733; 3,320,162; 3,312,618; 3,318,809; 3,471,403; 3,488,284; 3,595,790; and 3,629,109. The disclosures of these patents are hereby incorporated in this present specification for their disclosures in this regard as well as for their disclosure of specific suitable basic metal salts.

In the context of this invention, phenols are considered organic acids. Thus, overbased salts of phenols (generally known as phenates) are also useful in making (B-1) of this invention are well known to those skilled in the art. The phenols from which these phenates are formed are of the general formula:



(VII)

wherein  $R^*$ ,  $g$ ,  $Ar^*$ ,  $X$  and  $f$  have the same meaning and preferences are described hereinabove with reference to Formula III. The same examples described with respect to Formula III also apply.

A commonly available class of phenates are those made from phenols of the general formula:



(VIII)

wherein  $a^*$  is an integer of 1-3,  $b^*$  is 1 or 2,  $z^*$  is 0 or 1,  $R^{32}$  in Formula VIII is a hydrocarbyl-based substituent having an average of from 6 to about 400 aliphatic car-

bon atoms and  $R^{33}$  is selected from the group consisting of lower hydrocarbyl, lower alkoxyl, nitro, amino, cyano and halo groups.

One particular class of phenates for use in this invention are the overbased, Group IIA metal sulfurized phenates made by sulfurizing a phenol as described hereinabove with a sulfurizing agent such as sulfur, a sulfur halide, or sulfide or hydrosulfide salt. Techniques for making these sulfurized phenates are described in U.S. Pat. Nos. 2,680,096; 3,036,971; and 3,775,321 which are hereby incorporated by reference for their disclosures in this regard.

Other phenates that are useful are those that are made from phenols that have been linked through alkylene (e.g., methylene) bridges. These are made by reacting single or multi-ring phenols with aldehydes or ketones, typically, in the presence of an acid or basic catalyst. Such linked phenates as well as sulfurized phenates are described in detail in U.S. Pat. No. 3,350,038; particularly columns 6-8 thereof, which is hereby incorporated by reference for its disclosures in this regard.

Generally Group IIA overbased salts of the above-described carboxylic acids are typically useful in making (D-3) of this invention.

Component (D-3) may also be a borated complex of an overboard metal sulfonate, carboxylates or phenate. Borated complexes of this type may be prepared by heating the overboard metal sulfonate, carboxylate or phenate with boric acid at about 50°-100° C., the number of equivalents of boric acid being roughly equal to the number of equivalents of metal in the salt.

The method of preparing metal overbased compositions in this manner is illustrated by the following examples.

#### EXAMPLES (D)(8)-1

A mixture consisting essentially of 480 parts of a sodium petrosulfonate (average molecular weight of about 480), 84 parts of water, and 520 parts of mineral oil is heated at 100° C. The mixture is then heated with 86 parts of a 76% aqueous solution of calcium chloride and 72 parts of lime (90% purity) at 100° C. for two hours, dehydrated by heating to a water content of less than about 0.5%, cooled to 50° C., mixed with 130 parts of methyl alcohol, and then blown with carbon dioxide at 50° C. until substantially neutral. The mixture is then heated to 150° C. to distill off methyl alcohol and water and the resulting oil solution of the basic calcium sulfonate filtered. The filtrate is found to have a calcium sulfate ash content of 16% and a metal ratio of 2.5. A mixture of 1305 parts of the above carbonated calcium petrosulfonate, 930 parts of mineral oil, 220 parts of methyl alcohol, 72 parts of isobutyl alcohol, and 38 parts of amyl alcohol is prepared, heated to 35° C., and subjected to the following operating cycle four times: mixing with 143 parts of 90% commercial calcium hydroxide (90% calcium hydroxide) and treating the mixture with carbon dioxide until it has a base number of 32-39. The resulting product is then heated to 155° C. during a period of nine hours to remove the alcohol and filtered at this temperature. The filtrate is characterized by a calcium sulfate ash content of about 40% and a metal ratio of about 12.2.

#### EXAMPLE (D)(8)-2

A mineral oil solution of a basic, carbonated calcium complex is prepared by carbonating a mixture of an

alkylated benzene sulfonic acid (molecular weight of 470) an alkylated calcium phenate, a mixture of lower alcohols (methanol, butanol, and pentanol) and excess lime (5.6 equivalents per equivalent of the acid). The solution has a sulfur content of 1.7%, a calcium content of 12.6% and a base number of 336. To 950 grams of the solution, there is added 50 grams of a polyisobutene (molecular weight of 1000)-substituted succinic anhydride (having a saponification number of 100) at 25° C. The mixture is stirred, heated to 150° C., held at that temperature for 0.5 hour, and filtered. The filtrate has a base number of 315 and contains 35.4% of mineral oil.

#### EXAMPLE (D)(8)-3

A solution of 3192 parts (12 equivalents) of a 15 polyisobutene-substituted phenol, wherein the polyisobutene substituent has a molecular weight of about 175, in 2400 parts of mineral oil is heated to 70° C. and 502 parts (12 equivalents) of solid sodium hydroxide is added. The material is blown with nitrogen at 162° C. under vacuum to remove volatiles and is then cooled to 125° C. and 465 parts (12 equivalents) of 40% aqueous formaldehyde is added. The mixture is heated to 146° C. under nitrogen, and volatiles are finally removed again under vacuum. Sulfur dichloride, 618 parts (6 equivalents), is then added over 4 hours. Water, 1000 parts, is added at 70° C. and the mixture is heated to reflux for 1 hour. All volatiles are then removed under vacuum at 155° C. and the residue is filtered at that temperature, with the addition of a filter aid material. The filtrate is 30 the desired product (59% solution in mineral oil) containing 3.56% phenolic hydroxyl and 3.46% sulfur.

#### EXAMPLE (D)(8)-4

To a mixture of 3192 parts (12 equivalents) of tetra- 35 propenyl-substituted phenol, 2400 parts of mineral oil and 465 parts (6 equivalents) of 40% aqueous formaldehyde at 82° C., is added, over 45 minutes, 960 parts (12 equivalents) of 50% aqueous sodium hydroxide. Volatile materials are removed by stripping as in Example 40 (D)(8)-4, and to the residue is added 618 parts (12 equivalents) of sulfur dichloride over 3 hours. Toluene, 1000 parts, and 1000 parts of water are added and the mixture is heated under reflux for 2 hours. Volatile materials are then removed at 180° C. by blowing with nitrogen and the intermediate is filtered.

To 1950 parts (4 equivalents) of the intermediate thus obtained is added 135 parts of the polyisobutylene succinic anhydride of Example (D)(8)-2. The mixture is heated to 51° C., and 78 parts of acetic acid and 431 parts of methanol are added, followed by 325 parts (8.8 equivalents) of calcium hydroxide. The mixture is blown with carbon dioxide and is finally stripped with nitrogen blowing at 158° C. and filtered while hot, using a filter aid. The filtrate is a 68% solution in mineral oil of the desired product and contains 2.63% sulfur and 22.99% calcium sulfate ash.

#### EXAMPLE (D)(8)-5

A reaction mixture comprising about 512 parts by 60 weight of a mineral oil solution containing about 0.5 equivalent of a substantially neutral magnesium salt of an alkylated salicylic acid wherein the alkyl group has an average of about 18 aliphatic carbon atoms and about 30 parts by weight of an oil mixture containing about 0.037 equivalent of an alkylated benzenesulfonic acid together with about 15 parts by weight (about 0.65 equivalent) of a magnesium oxide and about 250 parts

by weight of xylene is added to a flask and heated to a temperature of about 60° C. to 70° C. The reaction mass is subsequently heated to about 85° C. and approximately 60 parts by weight of water are added. The 5 reaction mass is held at a reflux temperature of about 95° C. to 100° C. for about 1½ hours and subsequently stripped at a temperature of 155° C.-160° C., under a vacuum, and filtered. The filtrate comprises the basic carboxylic magnesium salt characterized by a sulfated ash content of 12.35% (ASTM D-874, IP 163), indicating that the salt contains 200% of the stoichiometrically equivalent amount of magnesium.

#### (D)(9) Carboxylic Dispersant Composition

The composition of the present invention comprises (D)(9) at least one carboxylic dispersant characterized by the presence within its molecular structure of (i) at least one polar group selected from acyl, acyloxy or hydrocarbyl-imidoyl groups, and (ii) at least one group in which a nitrogen or oxygen atom is attached directly to said group (i), and said nitrogen or oxygen atom also is attached to a hydrocarbyl group. The structures of the polar group (i), as defined by the International Union of Pure and Applied Chemistry, are as follows (R<sup>34</sup> representing a hydrocarbon or similar group):



Group (ii) is preferably at least one group in which a nitrogen or oxygen atom is attached directly to said polar group, said nitrogen or oxygen atom also being attached to a hydrocarbon group or substituted hydrocarbon group, especially an amino, alkylamino-, polyalkylene-amino-, hydroxy- or alkyleneoxy-substituted hydrocarbon group. With respect to group (ii), the dispersants are conveniently classified as "nitrogen-bridged dispersants" and "oxygen-bridged dispersants" 45 wherein the atom attached directly to polar group (i) is nitrogen or oxygen, respectively.

Generally, the carboxylic dispersants can be prepared by the reaction of a hydrocarbon-substituted succinic acid-producing compound (herein sometimes referred 50 to as the "succinic acylating agent") with at least about one-half equivalent, per equivalent of acid-producing compound, of an organic hydroxy compound, or an amine containing at least one hydrogen attached to a nitrogen group, or a mixture of said hydroxy compound and mine. The carboxylic dispersants (D)(9) obtained in this manner are usually complex mixtures whose precise composition is not readily identifiable. The nitrogen-containing carboxylic dispersants are sometimes referred to herein as "acylated amines". The compositions obtained by reaction of the acylating agent and alcohols are sometimes referred to herein as "carboxylic ester" dispersants. The carboxylic dispersants (D)(9) are either oil-soluble, or they are soluble in the oil-containing lubricating and functional fluids of this invention.

The soluble-nitrogen-containing carboxylic dispersants useful as component (D)(9) in the compositions of the present invention are known in the art and have been described in many U.S. patents including

|           |           |           |
|-----------|-----------|-----------|
| 3,172,892 | 3,341,542 | 3,630,904 |
| 3,219,666 | 3,444,170 | 3,787,374 |
| 3,272,746 | 3,454,607 | 4,234,435 |
| 3,316,177 | 3,541,012 |           |

The carboxylic ester dispersants useful as (D)(9) also have been described in the prior art. Examples of patents describing such dispersants include U.S. Pat. Nos. 3,381,022; 3,522,179; 3,542,678; 3,957,855; and 4,034,038. Carboxylic dispersants prepared by reaction of acylating agents with alcohols and amines or amino alcohols are described in, for example, U.S. Pat. Nos., 3,576,743 and 3,632,511.

The above U.S. patents are expressly incorporated herein by reference for their teaching of the preparation of carboxylic dispersants useful as component (D)(9).

One procedure for preparing (D)(9) useful in this invention is illustrated, in part, in U.S. Pat. No. 3,219,666 which is expressly incorporated herein by reference for its teachings in regard to preparing succinic acylating agents. This procedure is conveniently designated as the "two-step procedure". It involves first chlorinating the polyalkene until there is an average of at least about one chloro group for each molecular weight of polyalkene. (For purposes of this invention, the molecular weight of the polyalkene is the weight corresponding to the Mn value.) Chlorination involves merely contacting the polyalkene with chlorine gas until the desired amount of chlorine is incorporated into the chlorinated polyalkene. Chlorination is generally carried out at a temperature of about 75° C. to about 125° C. If a diluent is used in the chlorination procedure, it should be one which is not itself readily subject to further chlorination. Poly- and perchlorinated and/or fluorinated alkanes and benzenes are examples of suitable diluents.

The second step in the two-step chlorination procedure, for purposes of this invention, is to react the chlorinated polyalkene with the maleic reactant at a temperature usually within the range of about 100° C. to about 200° C. The mole ratio of chlorinated polyalkene to maleic reactant is usually about 1:1. (For purposes of this invention, a mole of chlorinated polyalkene is that weight of chlorinated polyalkene corresponding to the Mn value of the unchlorinated polyalkene.) However, a stoichiometric excess of maleic reactant can be used, for example, a mole ratio of 1:2. If an average of more than about one chloro group per molecule of polyalkene is introduced during the chlorination step, then more than one mole of maleic reactant can react per molecule of chlorinated polyalkene. Because of such situations, it is better to describe the ratio of chlorinated polyalkene to maleic reactant in terms of equivalents. (An equivalent weight of chlorinated polyalkene, for purposes of this invention, is the weight corresponding to the Mn value divided by the average number of chloro groups per molecule of chlorinated polyalkene while the equivalent weight of a maleic reactant is its molecular weight.) Thus, the ratio of chlorinated polyalkene to maleic reactant will normally be such as to provide about one equivalent of maleic reactant for each mole of chlorinated polyalkene up to about one equivalent of maleic reactant for each equivalent of chlorinated polyalkene with the understanding that it is normally desirable to provide an excess of maleic reactant; for example, an excess of about 5% to about 25% by weight. Unreacted excess maleic reactant may be stripped from the reac-

tion product, usually under vacuum, or reacted during a further stage of the process as explained below.

The resulting polyalkene-substituted succinic acylating agent is, optionally, again chlorinated if the desired number of succinic groups are not present in the product. If there is present, at the time of this subsequent chlorination, any excess maleic reactant from the second step, the excess will react as additional chlorine is introduced during the subsequent chlorination. Otherwise, additional maleic reactant is introduced during and/or subsequent to the additional chlorination step. This technique can be repeated until the total number of succinic groups per equivalent weight of substituent groups reaches the desired level.

Another procedure for preparing (D)(9) useful in this invention utilizes a process described in U.S. Pat. No. 3,912,764 and U.K. Patent 1,440,219, both of which are expressly incorporated herein by reference for their teachings in regard to that process. According to that process, the polyalkene and the maleic reactant are first reacted by heating them together in a "direct alkylation" procedure. When the direct alkylation step is completed, chlorine is introduced into the reaction mixture to promote reaction of the remaining unreacted maleic reactants. According to the patents, 0.3 to 2 or more moles of maleic anhydride are used in the reaction for each mole of olefin polymer; i.e., polyalkylene. The direct alkylation step is conducted at temperatures of 180°-250° C. During the chlorine-introducing stage, a temperature of 160°-225° C. is employed. In utilizing this process to prepare the substituted succinic acylating agents of this invention, it would be necessary to use sufficient maleic reactant and chlorine to incorporate at least 1.3 succinic groups into the final product for each equivalent weight of polyalkene.

Another process for preparing (D)(9) is the so-called "one-step" process. This process is described in U.S. Pat. Nos. 3,215,707 and 3,231,587. Both are expressly incorporated herein by reference from their teachings in regard to that process.

Basically, the one-step process involves preparing a mixture of the polyalkene and the maleic reactant containing the necessary amounts of both to provide the desired substituted succinic acylating agents of this invention. This means that there must be at least one mole of maleic reactant for each mole of polyalkene in order that there can be at least one succinic group for each equivalent weight of substituent groups. Chlorine is then introduced into the mixture, usually by passing chlorine gas through the mixture with agitation, while maintaining a temperature of at least about 140° C.

The amines which are reacted with the succinic acid-producing compounds to form the nitrogen-containing compositions (D)(9) may be monoamines and polyamines. The monoamines and polyamines must be characterized by the presence within their structure of at least one H—H<group. Therefore, they have at least one primary (i.e., H<sub>2</sub>N—) or secondary amino (i.e., 1H—N<) group. The amines can be aliphatic, cycloaliphatic, aromatic, or heterocyclic, including aliphatic-substituted cycloaliphatic, aliphatic-substituted aromatic, aliphatic-substituted heterocyclic, cycloaliphatic-substituted aliphatic, cycloaliphatic substituted aromatic, cycloaliphatic-substituted heterocyclic, aromatic-substituted aliphatic, aromatic-substituted cycloaliphatic, aromatic-substituted heterocyclic-substituted alicyclic, and heterocyclic-substituted aromatic amines

and may be saturated or unsaturated. The amines may also contain non-hydrocarbon substituents or groups as long as these groups do not significantly interfere with the reaction of the amines with the acylating reagents of this invention. Such non-hydrocarbon substituents or groups include lower alkoxy, lower alkyl mercapto, nitro, interrupting groups such as  $-\text{O}-$  and  $-\text{S}-$  (e.g., as in such groups as  $-\text{CH}_2\text{CH}_2-\text{X}-\text{CH}_2\text{CH}_2-$  where  $\text{X}$  is  $-\text{O}-$  or  $-\text{S}-$ ). In general, the mine of (D)(9) may be characterized by the formula



wherein  $\text{R}^{35}$  and  $\text{R}^{36}$  are each independently hydrogen or hydrocarbon, amino-substituted hydrocarbon, hydroxy-substituted hydrocarbon, alkoxy-substituted hydrocarbon, amino, carbamyl, thiocarbamyl, guanyl and acylimidoyl groups provided that only one of  $\text{R}^{35}$  and  $\text{R}^{36}$  may be hydrogen.

With the exception of the branched polyalkylene polyamine, the polyoxyalkylene polyamines, and the high molecular weight hydrocarbyl-substituted amines described more fully hereafter, the amines ordinarily contain less than about 40 carbon atoms in total and usually not more than about 20 carbon atoms in total.

Aliphatic monoamines include mono-aliphatic and di-aliphatic substituted amines wherein the aliphatic groups can be saturated or unsaturated and straight or branched chain. Thus, they are primary or secondary aliphatic amines. Such amines include, for example, mono- and di-alkyl-substituted amines, mono- and di-alkenyl-substituted amines, and amines having one N-alkenyl substituent and one N-alkyl substituent and the like. The total number of carbon atoms in these aliphatic monoamines will, as mentioned before, normally not exceed about 40 and usually not exceed about 20 carbon atoms. Specific examples of such monoamines include ethylamine, diethylamine, n-butylamine, di-n-butylamine, allylamine, isobutylamine, cocoamine, stearylamine, laurylamine, methylaurylamine, oleyl-amine, N-methyl-octylamine, dodecylamine, octadecyl-amine, and the like. Examples of cycloaliphatic-substituted aliphatic amines, aromatic-substituted aliphatic amines, and heterocyclic-substituted aliphatic amines, include 2-(cyclohexyl)-ethylamine, benzylamine, phenethylamine, and 3-(furylpropyl) amine.

Cycloaliphatic monoamines are those monoamines wherein there is one cycloaliphatic substituent attached directly to the amino nitrogen through a carbon atom in the cyclic ring structure. Examples of cycloaliphatic monoamines include cyclohexylamines, cyclopentylamines, cyclohexenylamines, cyclopentenylamines, N-ethyl-cyclohexylamine, dicyclohexylamines, and the like. Examples of aliphatic-substituted, aromatic-substituted, and heterocyclic-substituted cycloaliphatic monoamines include propyl-substituted cyclohexylamines, phenyl-substituted cyclopentylamines, and pyranyl-substituted cyclohexylamine.

Aromatic amines include those monoamines wherein a carbon atom of the aromatic ring structure is attached directly to the amino nitrogen. The aromatic ring will usually be a mononuclear aromatic ring (i.e., one derived from benzene) but can include fused aromatic rings, especially those derived from naphthalene. Examples of aromatic monoamines include aniline, di-(paramethyl-phenyl)amine, naphthylamine, N,N-dibutyl aniline, and the like. Examples of aliphatic-substituted, cycloaliphatic-substituted, and heterocyclic-substituted aromatic monoamines are para-ethoxyani-

line, para-dodecylaniline, cyclohexyl-substituted naphthylamine, and thietyl-substituted aniline.

The polyamines from which (D)(9) is derived include principally alkylene amines conforming for the most part to the formula



10

wherein  $t$  is an integer preferably less than about 10, A is a hydrogen group or a substantially hydrocarbon group preferably having up to about 30 carbon atoms, and the alkylene group is preferably a lower alkylene group having less than about 8 carbon atoms. The alkylene amines include principally methylene amines, ethylene amines, hexylene amines, heptylene amines, octylene amines, other polymethylene amines. They are exemplified specifically by: ethylene diamine, triethylene tetramine, propylene diamine, decamethylene diamine, octamethylene diamine, di(heptamethylene) triamine, tripropylene tetramine, tetraethylene pentamine, trimethylene diamine, pentaethylene hexamine, di(trimethylene) triamine. Higher homologues such as are obtained by condensing two or more of the above-illustrated alkylene amines likewise are useful.

The ethylene amines are especially useful. They are described in some detail under the heading "Ethylene Amines" in Encyclopedia of Chemical Technology, Kirk and Othmer, Vol. 5, pp. 898-905, Interscience Publishers, New York (1950). Such compounds are prepared most conveniently by the reaction of an alkylene chloride with ammonia. The reaction results in the production of somewhat complex mixtures of alkylene amines, including cyclic condensation products such as piperazines. These mixtures find use in the process of this invention. On the other hand, quite satisfactory products may be obtained also by the use of pure alkylene amines. An especially useful alkylene amine for reasons of economy as well as effectiveness of the products derived therefrom is a mixture of ethylene amines prepared by the reaction of ethylene chloride and ammonia and having a composition which corresponds to that of tetraethylene pentamine.

Hydroxyalkyl-substituted alkylene amines, i.e., alkylene amines having one or more hydroxyalkyl substituents on the nitrogen atoms, likewise are contemplated for use herein. The hydroxyalkyl-substituted alkylene amines are preferably those in which the alkyl group is a lower alkyl group, i.e., having less than about 6 carbon atoms. Examples of such amines include N-(2-hydroxyethyl)ethylene diamine, N,N'-bis(2-hydroxy-ethyl)-ethylene diamine, 1(2-hydroxyethyl)piperazine, mono-hydroxypropyl)piperazine, di-hydroxypropyl-substituted tetraethylene pentamine, N-(3-hydroxypropyl)-tetra-methylene diamine, and 2-heptadecyl-(2-hydroxyethyl)-imidazoline.

The nitrogen-containing composition (D)(9) obtained by reaction of the succinic acid-producing compounds and the amines described above may be amine salts, amides, imides, imidazolines as well as mixtures thereof. To prepare the nitrogen-containing composition (D)(9), one or more of the succinic acid-producing compounds and one or more of the amines are heated, optionally in the presence of a normally liquid, substantially inert organic liquid solvent/diluent at an elevated temperature generally in the range of from about 80° C. up to

the decomposition point of the mixture or the product. Normally, temperatures in the range of about 100° C. up to about 300° C. are utilized provided that 300° C. does not exceed the decomposition point.

The succinic acid-producing compound and the amine are reacted in mounts sufficient to provide at least about one-half equivalent, per equivalent of acid-producing compound, of the amine. Generally, the maximum amount of amine present will be about 2 moles of amine per equivalent of succinic acid-producing compound. For the purposes of this invention, an equivalent of the amine is that amount of the amine corresponding to the total weight of amine divided by the total number of nitrogen atoms present. Thus, octyl amine has an equivalent weight equal to its molecular weight; ethylene diamine has an equivalent weight equal to one-half its molecular weight; and aminoethyl piperazine has an equivalent weight equal to one-third its molecular weight. The number of equivalents of succinic acid-producing compound will vary with the number of succinic groups present therein, and generally, there are two equivalents of acylating reagent for each succinic group in the acylating reagents. Conventional techniques may be used to determine the number of carboxyl functions (e.g., acid number, saponification number) and, thus, the number of equivalents of acylating reagent available to react with amine. Additional details and examples of the procedures for preparing the nitrogen-containing compositions of the present invention by reaction of succinic acid-producing compounds and amines are included in, for example, U.S. Pat. Nos. 3,172,892; 3,219,666; 3,272,746; and 4,234,435, the disclosures of which are hereby incorporated by reference.

The following example is illustrative of the process for preparing the carboxylic dispersant compositions useful in this invention:

#### EXAMPLE (D)(9)-1

A polyisobutetyl succinic anhydride is prepared by 40 the reaction of a chlorinated polyisobutylene with maleic anhydride at 200° C. The polyisobutetyl group has an average molecular weight of 850 and the resulting alkenyl succinic anhydride is found to have an acid number of 113 (corresponding to an equivalent weight of 500). To a mixture of 500 grams (1 equivalent) of this polyisobutetyl succinic anhydride and 160 grams of toluene there is added at room temperature 35 grams (1 equivalent) of diethylene triamine. The addition is made portionwise throughout a period of 15 minutes, and an initial exothermic reaction caused the temperature to rise to 50° C. The mixture then is heated and a water-toluene azeotrope distilled from the mixture. When no more water distills, the mixture is heated to 150° C. at reduced pressure to remove the toluene. The residue is 55 diluted with 350 grams of mineral oil and this solution is found to have a nitrogen content of 1.6%.

#### (D)(10) The Nitrogen-Containing Organic Composition

A nitrogen-containing organic composition may be utilized comprising

- (a) an acylated, nitrogen containing compound having a substituent of at least 10 aliphatic carbon atoms made by reacting a carboxylic acylating agent with at least one amino compound containing at least one —NH group, said acylating agent being 65 linked to said amino compound through an imido, amido, amidine or acyloxy ammonium linkage, and
- (b) at least one amino phenol of the general formula



wherein R<sup>37</sup> is a substantially saturated, hydrocarbon-based substituent of at least 10 aliphatic carbon atoms; a, b and c are each independently an integer of one up to three times the number of aromatic nuclei present in Ar with the proviso that the sum of a, b and c does not exceed the unsaturated valences of Ar; and Ar is an aromatic moiety having 0-3 optional substituents selected from the group consisting of lower alkyl, lower alkoxy, nitro, halo or combinations of two or more of said substituents.

Within the nitrogen-containing organic composition, the weight ratio of (a):(b) is from (50-95):(50-5), preferably (50-75):(50-25) and most preferably from (50-60):(50-40).

A number of acylated, nitrogen-containing compounds having a substituent R<sup>37</sup> of at least 10 aliphatic carbon atoms and made by reacting a carboxylic acid acylating agent with an amino compound are known to those skilled in the art. In such compositions the acylating agent is linked to the amino compound through an imidazoline imido, amido, amidine or acyloxy ammonium linkage. The substituent of 10 aliphatic carbon atoms, preferably 30 aliphatic carbon atoms, may be in either the carboxylic acid acylating agent derived portion of the molecule or in the amino compound derived portion of the molecule. Preferably, however, it is in the acylating agent portion. The acylating agent can vary from formic acid and its acylating derivatives to acylating agents having high molecular weight aliphatic substituents of up to 5,000, 10,000 or 20,000 carbon atoms. The amino compounds can vary from ammonia itself to amines having aliphatic substituents of up to about 30 carbon atoms. A more detailed discussion of the substantially saturated, hydrocarbon-based substituent R<sup>37</sup> can be found in U.S. Pat. No. 4,724,091 which is herein incorporated by reference.

A typical class of acylated amino compounds useful in making the compositions of this invention are those made by reacting an acylating agent having an aliphatic substituent of at least 10 carbon atoms and a nitrogen compound characterized by the presence of at least one —NH group. Typically, the acylating agent will be a mono- or polycarboxylic acid (or reactive equivalent thereof) such as a substituted succinic or propionic acid and the amino compound will be a polyamine or mixture of polyamines, most typically, a mixture of ethylene polyamines. The aliphatic substituent R<sup>37</sup> in such acylating agents is often of at least about 50 and up to about 400 carbon atoms. The aliphatic substituted R<sup>37</sup> is derived from homopolymerized or interpolymerized C<sub>2-10</sub> 1-olefins or mixtures of both. Usually R<sup>37</sup> is derived from ethylene, propylene, butylene and mixtures thereof. Typically, it is derived from polymerized isobutene. Exemplary of amino compounds useful in making these acylated compounds are the following:

- (1) polyalkylene polyamines of the general formula



Formula IX

wherein each  $R^{38}$  is independently a hydrogen atom, a lower alkyl group, a lower hydroxy alkyl group or a  $C_{1-12}$  hydrocarbon-based group, with the proviso that at least one  $R^{38}$  is a hydrogen atom,  $n$  is a whole number of 1 to 10 and  $U$  is a  $C_{2-10}$  alkylene group, (2) heterocyclic-substituted polyamines of the formula



wherein  $R^{38}$  and  $U$  are as defined hereinabove,  $m$  is 0 or a whole number of 1 to 10,  $m'$  is a whole number of 1 to 10 and  $Y$  is an oxygen or divalent sulfur atom or a  $N-R^{41}$  group and (3) aromatic polyamines of the general formula



wherein  $Ar$  is an aromatic nucleus of 6 to about 20 carbon atoms, each  $R^{38}$  is as defined hereinabove and  $y$  is 2 to about 8. Specific examples of the polyalkylene polyamines (1) are ethylene diamine, tetra(ethylene)-pentamine, tri(trimethylene)tetramine, 1,2-propylene diamine, etc. Specific examples of the heterocyclic-substituted polyamines (2) are  $N$ -2-aminoethyl piperazine,  $N$ -2 and  $N$ -3 amino propyl morpholine,  $N$ -3-(dimethyl amino) propyl piperazine, etc. Specific examples of the aromatic polyamines (3) are the various isomeric phenylene diamines, the various isomeric naphthylene diamines, etc.

Many patents have described useful acylated nitrogen compounds including U.S. Pat. Nos. 3,172,892; 3,219,666; 3,272,746; 3,310,492; 3,341,542; 3,444,170; 3,455,831; 3,455,832; 3,576,743; 3,630,904; 3,632,511; and 3,804,763. A typical acylated nitrogen-containing compound of this class is that made by reacting a poly(isobutene)-substituted succinic anhydride acylating agent (e.g., anhydride, acid, ester, etc.) wherein the poly(isobutene) substituent has between about 50 to about 400 carbon atoms with a mixture of ethylene polyamines having 3 to about 7 amino nitrogen atoms per ethylene polyamine and about 1 to about 6 ethylene units made from condensation of ammonia with ethylene chloride. In view of the extensive disclosure of this type of acylated amino compound, further discussion of their nature and method of preparation is not needed here. Instead, the above-noted U.S. Patents are hereby incorporated by reference for their disclosure of acylated amino compounds and their method of preparation.

Another type of acylated nitrogen compound belonging to this class is that made by reacting the aforescribed alkylene amines with the aforescribed substituted succinic acids or anhydrides and aliphatic monocarboxylic acids having from 2 to about 22 carbon atoms. In these types of acylated nitrogen compounds, the mole ratio of succinic acid to mono-carboxylic acid ranges from about 1:0.1 to about 1:1. Typical of the mono-carboxylic acid are formic acid, acetic acid, dodecanoic acid, butanoic acid, oleic acid, stearic acid, the commercial mixture of stearic acid isomers known as isostearic acid, tolyl acid, etc. Such materials are more fully described in U.S. Pat. Nos. 3,216,936 and 3,250,715 which are hereby incorporated by reference for their disclosures in this regard.

Still another type of acylated nitrogen compound is the product of the reaction of a fatty monocarboxylic acid of about 12-30 carbon atoms and the afores-

cribed alkylene amines, typically, ethylene, propylene or trimethylene polyamines containing 2 to 8 amino groups and mixtures thereof. The fatty monocarboxylic acids are generally mixtures of straight and branched chain fatty carboxylic acids containing 12-30 carbon atoms. A widely used type of acylated nitrogen compound is made by reacting the aforescribed alkylene polyamines with a mixture of fatty acids having from 5 to about 30 mole percent straight chain acid and about 70 to about 95 percent mole branched chain fatty acids. Among the commercially mailable mixtures are those known widely in the trade as isostearic acid. These mixtures are produced as a by-product from the dimerization of unsaturated fatty acids as described in U.S. Pat. Nos. 2,812,342 and 3,260,671.

The branched chain fatty acids can also include phenyl and cyclohexyl stearic acid and the chlorostearic acids. Branched chain fatty carboxylic acid/alkylene polyamine products have been described extensively in the art. See for example, U.S. Pat. Nos. 3,110,673; 3,251,853; 3,326,801; 3,337,459; 3,405,064; 3,429,674; 3,468,639; 3,857,791. These patents are hereby incorporated by reference for their disclosure of fatty acid/polyamine condensates and their use in lubricating oil formulations.

The aromatic moiety,  $Ar$ , of the amino phenol can be a single aromatic nucleus such as a benzene nucleus, a pyridine nucleus, a thiophene nucleus, a 1,2,3,4-tetrahydronaphthalene nucleus, etc., or a polynuclear aromatic moiety. Such polynuclear moieties can be of the fused type; that is, wherein at least one aromatic nucleus is fused at two points to another nucleus such as found in naphthalene, anthracene, the azanaphthalenes, etc. Alternatively, such polynuclear aromatic moieties can be of the linked type wherein at least two nuclei (either mono- or polynuclear) are linked through bridging linkages to each other. Such bridging linkages can be chosen from the group consisting of carbon-to-carbon single bonds, ether linkages, keto linkages, sulfide linkages, polysulfide linkages of 2 to 6 sulfur atoms, sulfonyl linkages, sulfonyl linkages, methylene linkages, alkylene linkages, di-(lower alkyl)methylene linkages, lower alkylene ether linkages, alkylene keto linkages, lower alkylene sulfur linkages, lower alkylene polysulfide linkages of 2 to 6 carbon atoms, amino linkages, polyamino linkages and mixtures of such divalent bridging linkages. In certain instances, more than one bridging linkage can be present in  $Ar$  between aromatic nuclei. For example, a fluorene nucleus has two benzene nuclei linked by both a methylene linkage and a covalent bond. Such a nucleus may be considered to have 3 nuclei but only two of them are aromatic. Normally, however,  $Ar$  will contain only carbon atoms in the aromatic nuclei per se (plus any lower alkyl or alkoxy substituent present).

The number of aromatic nuclei, fused, linked or both, in  $Ar$  can play a role in determining the integer values of  $a$ ,  $b$  and  $c$  of the amino phenol. For example, when  $Ar$  contains a single aromatic nucleus,  $a$ ,  $b$  and  $c$  are each independently 1 to 4. When  $Ar$  contains two aromatic nuclei,  $a$ ,  $b$  and  $c$  can each be an integer of 1 to 8, that is, up to three times the number of aromatic nuclei present (in naphthalene, 2). With a tri-nuclear  $Ar$  moiety,  $a$ ,  $b$  and  $c$  can each be an integer of 1 to 12. For example, when  $Ar$  is a biphenyl or a naphthyl moiety,  $a$ ,  $b$  and  $c$  can each independently be an integer of 1 to 8. The values of  $a$ ,  $b$  and  $c$  are obviously limited by the fact

that their sum cannot exceed the total unsatisfied valences of Ar.

The single ring aromatic nucleus which can be the Ar moiety can be represented by the general formula



wherein ar represents a single ring aromatic nucleus (e.g., benzene) of 4 to 10 carbons, each Q independently represents a lower alkyl group, lower alkoxy group, nitro group, or halogen atom, and m is 0 to 3. As used in this specification and appended claims, "lower" refers to groups having 7 or less carbon atoms such as lower alkyl and lower alkoxy groups. Halogen atoms include fluorine, chlorine, bromine and iodine atoms; usually, the halogen atoms are fluorine and chlorine atoms. As will be appreciated from inspection of the amino phenol formula, it contains at least one of each of the following substituents: a hydroxyl group, a R<sup>30</sup> group as defined above, and a primary amine group, —NH<sub>2</sub>. Each of the foregoing groups must be attached to a carbon atom which is a part of an aromatic nucleus in the Ar moiety. They need not, however, each be attached to the same aromatic ring if more than one aromatic nucleus is present in the Ar moiety.

In a preferred embodiment, the amino phenols contain one each of the foregoing substituents (i.e., a, b and c are each 1) and but a single aromatic ring, most preferably benzene. This preferred class of amino phenols can be represented by the formula



Formula XII

wherein the R<sup>39</sup> group is a substantially saturated hydrocarbon-based group of about 30 to about 400 aliphatic carbon atoms located ortho or para to the hydroxyl group, R<sup>40</sup> is a lower alkyl, lower alkoxy, nitro group or halogen atom and z is O or 1. Usually z is 0 and R<sup>39</sup> is a substantially saturated, purely hydrocarbyl aliphatic group. Often it is an alkyl or alkenyl group para to the —OH substituent. Often there is but one amino group, —NH<sub>2</sub> in these preferred amino phenols but there can be two.

In a still more preferred embodiment, the amino phenol is of the formula



Formula XIII

wherein R<sup>41</sup> is derived from homopolymerized or interpolymerized C<sub>2</sub>-10 1-olefins and has an average of from about 30 to about 400 aliphatic carbon atoms and R<sup>40</sup> and z are as defined above. Usually R<sup>41</sup> is derived from ethylene, propylene, butylene and mixtures thereof. Typically, it is derived from polymerized isobutene. Often R<sup>41</sup> has at least about 50 aliphatic carbon atoms and z is zero.

The amino phenols can be prepped by a number of synthetic routes. These routes can vary in the type reactions used and the sequence in which they are employed. For example, an aromatic hydrocarbon, such as benzene, can be alkylated with alkylating agent such as a polymeric olefin to form an alkylated aromatic intermediate. This intermediate can then be nitrated, for example, to form polynitro intermediate. The polynitro intermediate can in turn be reduced to a diamine, which can then be diazotized and reacted with water to convert one of the amino groups into a hydroxyl group and provide the desired amino phenol. Alternatively, one of the nitro groups in the polynitro intermediate can be converted to a hydroxyl group through fusion with caustic to provide a hydroxy-nitro alkylated aromatic which can then be reduced to provide the desired amino phenol.

Another useful route to the amino phenols involves the alkylation of a phenol with an olefinic alkylating agent to form an alkylated phenol. This alkylated phenol can then be nitrated to form an intermediate nitro phenol which can be converted to the desired amino phenols by reducing at least some of the nitro groups to amino groups.

Typically the amino phenols are obtained by reduction of nitro phenols with hydrogen in the presence of a metallic catalyst such as discussed above. This reduction is generally carried out at temperatures of about 15°-250° C., typically, about 50°-150° C., and hydrogen pressures of about 0-2000 psig, typically, about 50-250 psig. The reaction time for reduction usually varies between about 0.5-50 hours. Substantially inert liquid diluents and solvents, such as ethanol, cyclohexane, etc., can be used to facilitate the reaction. The amino phenol product is obtained by well-known techniques such as distillation, filtration, extraction, and so forth.

The reduction is carried out until at least about 50%, usually about 80%, of the nitro groups present in the nitro intermediate mixture are converted to amino groups. The typical route to the amino phenols just described can be summarized as

(I) nitrating with at least one nitrating agent at least one compound of the formula



Formula XIV

wherein R<sup>42</sup> is a substantially saturated hydrocarbon-based group of at least 10 aliphatic carbon atoms; a and c are each independently an integer of 1 up to three times the number of aromatic nuclei present in Ar' with the proviso that the sum of a, b and c does not exceed the unsatisfied valences of Ar'; and Ar' is an aromatic moiety having 0 to 3 optional substituents selected from the group consisting of lower alkyl, lower alkoxy, nitro, and halo, or combinations of two or more optional substituents, with the provisos that (a) Ar' has at least one hydrogen atom directly bonded to a carbon atom which is part of an aromatic nucleus, and (b) when Ar' is a benzene having only one hydroxyl and one R substituent, the R substituent is ortho or para to said hydroxyl substituent, to form a first reaction mixture containing a nitro intermediate, and (II) reducing at least about 50% of the nitro groups in said first reaction mixture to amino groups.

Usually this means reducing at least about 50% of the nitro groups to amino groups in a compound or mixture of compounds of the formula



Formula XV

wherein  $\text{R}^{42}$  is a substantially saturated hydrocarbon-based substituent of at least 10 aliphatic carbon atoms;  $a$ ,  $b$  and  $c$  are each independently an integer of 1 up to three times the number of aromatic nuclei present in  $\text{Ar}$  with the proviso that the sum of  $a$ ,  $b$  and  $c$  does not exceed the unsatisfied valences of  $\text{Ar}$ ; and  $\text{Ar}$  is an aromatic moiety having 0 to 3 optional substituents selected from the group consisting of lower alkyl, lower alkoxy, halo, or combinations of two or more of said optional substituents; with the proviso that when  $\text{Ar}$  is a benzene nucleus having only one hydroxyl and one  $\text{R}$  substituent, the  $\text{R}^{42}$  substituent is ortho or para to said hydroxyl substituent.

The following specific illustrative examples describe how to make the nitrogen-containing organic compositions. In these examples, as well as in this specification and the appended claims, all percentages, parts and ratios are by weight, unless otherwise expressly stated to the contrary. Temperatures are in degrees centigrade ( $^{\circ}\text{C}$ ) unless expressly stated to the contrary.

#### EXAMPLE (D)(10)a-1

To 1,133 parts of commercial diethylene triamine heated at  $110^{\circ}$ - $150^{\circ}$  is slowly added 6820 parts of isostearic acid over a period of two hours. The mixture is held at  $150^{\circ}$  for one hour and then heated to  $180^{\circ}$  over an additional hour. Finally, the mixture is heated to  $205^{\circ}$  over 0.5 hour; throughout this heating, the mixture is blown with nitrogen to remove volatiles. The mixture is held at  $205^{\circ}$ - $230^{\circ}$  for a total of 11.5 hours and then stripped at  $230^{\circ}$ /20 torr to provide the desired acylated polyamine as a residue containing 6.2% nitrogen.

#### EXAMPLE (1)(10)b-1

A mixture of 4578 parts of a polyisobutene-substituted phenol prepared by boron trifluoride-phenol catalyzed alkylation of phenol with a polyisobutene having a number average molecular weight of approximately 1000 (vapor phase osmometry), 3052 parts of diluent mineral oil and 725 parts of textile spirits is heated to  $60^{\circ}$  to achieve homogeneity. After cooling to  $30^{\circ}$ , 319.5 parts of 16 molar nitric acid in 600 parts of water is added to the mixture. Cooling is necessary to keep the mixture's temperature below  $40^{\circ}$ . After the reaction mixture is stirred for an additional two hours, an aliquot of 3,710 parts is transferred to a second reaction vessel. This second portion is treated with an additional 127.8 parts of 16 molar nitric acid in 130 parts of water at  $25^{\circ}$ - $30^{\circ}$ . The reaction mixture is stirred for 1.5 hours and then stripped to  $220^{\circ}$ /30 torr. Filtration provides an oil solution of the desired intermediate (D)(10)b-1.

#### EXAMPLE (D)(10)b-2

A mixture of 810 parts of the oil solution of the (D)(10)b-1 intermediate described in Example (D)(10)b-1, 1,405 parts of isopropyl alcohol and 405 parts of toluene is charged to an appropriately sized autoclave. Platinum oxide catalyst (0.81 part) is added and the autoclave evacuated and purged with nitrogen four times to remove any residual air. Hydrogen is fed to the autoclave

at a pressure of 29-55 psig while the content is stirred and heated to  $27^{\circ}$ - $92^{\circ}$  for a total of thirteen hours. Residual excess hydrogen is removed from the reaction mixture by evacuation and purging with nitrogen four times. The reaction mixture is then filtered through diatomaceous earth and the filtrate stripped to provide an oil solution of the desired amino phenol. This solution contains 0.578% nitrogen.

#### (D)(11) The Zinc Salt

A zinc salt of the formula



wherein  $\text{R}^{43}$  and  $\text{R}^{44}$  are independently hydrocarbyl groups containing from about 3 to about 20 carbon atoms are readily obtainable by the reaction of phosphorus pentasulfide ( $\text{P}_2\text{S}_5$ ) and an alcohol or phenol. The reaction involves mixing at a temperature of about  $20^{\circ}$  C. to about  $200^{\circ}$  C., four moles of an alcohol or a phenol with one mole of phosphorus pentasulfide. Hydrogen sulfide is liberated in this reaction.

The  $\text{R}^{43}$  ad  $\text{R}^{44}$  groups are independently hydrocarbyl groups that are preferably free from acetylenic and usually also from ethylenic unsaturation and have from about 3 to about 20 carbon atoms, preferably 3 to about 16 carbon atoms and most preferably 3 to about 12 carbon atoms.

#### EXAMPLE (D)(11)-1

A reaction mixture is prepared by the addition of 3120 parts (24.0 moles) of 2-ethylhexanol and 444 parts (6.0 moles) of isobutyl alcohol. With nitrogen blowing at 1.0 cubic feet per hour, 1540 parts (6.9 moles) of  $\text{P}_2\text{S}_5$  is added to the mixture over a two-hour period while maintaining the temperature at  $60^{\circ}$ - $78^{\circ}$  C. The mixture is held at  $75^{\circ}$  C. for one hour and stirred an additional two hours while cooling. The mixture is filtered through diatomaceous earth. The filtrate is the product. (D)(12) The Sulfurized Composition

Within the purview of this invention, two different sulfurized compositions are envisaged and have utility. The first sulfurized composition, is a sulfurized olefin prepared by reacting an olefin/sulfur halide complex by contacting the complex with a protic solvent in the presence of metal ions at a temperature in the range of  $40^{\circ}$  C. to  $120^{\circ}$  C. and thereby removing halogens from the sulfurized complex and providing a dehalogenated sulfurized olefin; and isolating the sulfurized olefin.

The preparation of the first sulfurized composition generally involves reacting an olefin with a sulfur halide to obtain an alkyl/sulfur halide complex, a sulfochlorination reaction. This complex is contacted with metal ions and a protic solvent. The metal ions are in the form of  $\text{Na}_2\text{S}/\text{NaSH}$  which is obtained as an effluent of process streams from hydrocarbons, additional  $\text{Na}_2\text{S}$  and  $\text{NaOH}$ . The  $\text{Na}_2\text{S}/\text{NaSH}$  may also be in the form of a fresh solution, that is, not recycled. The protic solvent is water and an alcohol of 4 carbon atoms or less. Preferably, the alcohol is isopropyl alcohol. The reaction with the metal ions and protic solvent represents a sulfurization-dechlorination reaction. The metal ions are present in an aqueous solution. The metal ions solution is pre-

pared by blending an aqueous  $\text{Na}_2\text{S}$  solution with the  $\text{Na}_2\text{S}/\text{NaSH}$  process streams. Water and aqueous  $\text{NaOH}$  are added as necessary to adjust the  $\text{Na}_2\text{S}$  and  $\text{NaOH}$  concentration to a range of 18-21%  $\text{Na}_2\text{S}$  and 2-5%  $\text{NaOH}$ . A sulfurized product is obtained which is substantially free of any halide, i.e. the product obtained has had enough of the halide removed so that it is useful as a lubricant additive. U.S. Pat. No. 4,764,297 is incorporated herein by reference for its disclosure of this first sulfurized composition.

The following example is provided so as to provide those of ordinary skill in the art with a complete disclosure and description of how to make the first sulfurized composition.

#### EXAMPLE (D)(12)-1

Added to a three-liter, four-necked flask are 1100 grams (8.15 moles) of sulfur monochloride. While stirring at room temperature 952 grams (17 moles) of isobutylene are added below the surface. The reaction is 20 exothermic and the addition rate of isobutylene controls the reaction temperature. The temperature is allowed to reach a maximum of 50° C. and obtained is a sulfochlorination reaction product.

A blend of 1800 grams of 18%  $\text{Na}_2\text{S}$  solution is obtained from process streams. To this blend is added 238 grams 50% aqueous  $\text{NaOH}$ , 525 grams water and 415 grams isopropyl alcohol to prepare a reagent for use in the sulfurization-dechlorination reaction. To this reagent is added 1000 grams of the sulfochlorination reaction product in about 1.5 hours. One hour after the addition is completed, the contents are permitted to settle and the liquid layer is drawn off and discarded. The organic layer is stripped to 120° C. and 100 mm Hg to remove any volatiles. Analyses: % sulfur 43.5, % 35 chlorine 0.2.

Table I outlines other olefins and sulfur chlorides that can be utilized in preparing the first sulfurized composition. The procedure is essentially the same as in Example (D)(12)-1. In all the examples, the metal ion reagent is prepared according to Example (D)(12)-1.

TABLE I

| Example    | Olefin                                  | Sulfur Chloride         | Mole Ratio of Olefin:SCl |
|------------|-----------------------------------------|-------------------------|--------------------------|
| (D)(12)-2  | n-butene                                | $\text{S}\text{Cl}_2$   | 2.3:1                    |
| (D)(12)-3  | propene                                 | $\text{S}_2\text{Cl}_2$ | 2.5:1                    |
| (D)(12)-4  | n-pentene                               | $\text{S}_2\text{Cl}_2$ | 2.2:1                    |
| (D)(12)-5  | n-butene/<br>isobutylene<br>1:1 weight  | $\text{S}_2\text{Cl}_2$ | 2.5:1                    |
| (D)(12)-6  | isobutylene/<br>2-pentene<br>1:1 weight | $\text{S}_2\text{Cl}_2$ | 2.2:1                    |
| (D)(12)-7  | isobutylene/<br>2-pentene<br>3:2 weight | $\text{S}_2\text{Cl}_2$ | 2.2:1                    |
| (D)(12)-8  | isobutylene/<br>propene<br>6:1 weight   | $\text{S}_2\text{Cl}_2$ | 2.3:1                    |
| (D)(12)-9  | n-pentene/<br>2-pentene<br>1:1 weight   | $\text{S}_2\text{Cl}_2$ | 2.2:1                    |
| (D)(12)-10 | 2-pentene/<br>propene<br>3:2 weight     | $\text{S}_2\text{Cl}_2$ | 2.2:1                    |

The second sulfurized composition is an oil-soluble sulfur-containing material which comprises the reaction product of sulfur and a Diels-Alder adduct. The Diels-Alder adducts are a well-known, art-recognized class of compounds prepared by the diene synthesis or Diels-

Alder reaction. A summary of the prior art relating to this class of compounds is found in the Russian monograph, *Dienovy Sintez*, Izdatelstwo Akademii Nauk SSSR, 1963 by A. S. Onischenko. (Translated into the English language by L. Mandel as A. S. Onischenko, *Diene Synthesis*, New York, Daniel Davey and Co., Inc., 1964) This monograph and references cited therein are incorporated by reference into the present specification.

Basically, the diene synthesis (Diels-Alder reaction) involves the reaction of at least one conjugated diene,  $>\text{C}=\text{C}-\text{C}=<$ , with at least one ethylenically or acetylenically unsaturated compound,  $>\text{C}=\text{C}<$ , these latter compounds being known as dienophiles. The reaction can be represented as follows:

Reaction 1:



Reaction 2:



The products, A and B are commonly referred to as Diels-Alder adducts. It is these adducts which are used as starting materials for the preparation of the second sulfurized composition.

Representative examples of such 1,3-dienes include aliphatic conjugated diolefins or dienes of the formula



wherein  $\text{R}^{45}$  through  $\text{R}^{50}$  are each independently selected from the group consisting of halogen, alkyl, halo, alkoxy, alkenyl, alkenyloxy, carboxy, cyano, amino, alkylamino, dialkylamino, phenyl, and phenyl-substituted with 1 to 3 substituents corresponding to  $\text{R}^{45}$  through  $\text{R}^{50}$  with the proviso that a pair of R's on adjacent carbons do not form an additional double bond in the diene. Preferably not more than three of the R variables are other than hydrogen and at least one is hydrogen. Normally the total carbon content of the diene will not exceed 20. U.S. Pat. No. 4,582,618 is incorporated herein by reference for its disclosure of this second sulfurized composition.

The adducts and processes of preparing the adducts are further exemplified by the following examples. Unless otherwise indicated in these examples and in other parts of this specification, as well as in the appended claims, all parts and percentages are by weight.

## EXAMPLE A

A mixture comprising 400 parts of toluene and 66.7 parts of aluminum chloride is charged to a two-liter flask fitted with a stirrer, nitrogen inlet tube, and a solid carbon dioxide-cooled reflux condenser. A second mixture comprising 640 parts (5 moles) of butyl acrylate and 240.8 parts of toluene is added to the  $\text{Al Cl}_3$  slurry while maintaining the temperature within the range of 37°–58° C. over a 0.25-hour period. Thereafter, 313 parts (5.8 moles) of butadiene is added to the slurry over a 2.75-hour period while maintaining the temperature of the reaction mass at 50°–61° C. by means of external cooling. The reaction mass is blown with nitrogen for about 0.33 hour and then transferred to a four-liter separatory funnel and washed with a solution of 150 parts of concentrated hydrochloric acid in 1100 parts of water. Thereafter, the product is subjected to two additional water washings using 1000 parts of water for each wash. The washed reaction product is subsequently distilled to remove unreacted butyl acrylate and toluene. The residue of this first distillation step is subjected to further distillation at a pressure of 9–10 millimeters of mercury whereupon 785 parts of the desired product is collected over the temperature of 105°–115° C.

## EXAMPLE B

The adduct of isoprene and acrylonitrile is prepared by mixing 136 parts of isoprene, 106 parts of acrylonitrile, and 0.5 parts of hydroquinone (polymerization inhibitor) in a rocking autoclave and thereafter heating for 16 hours at a temperature within the range of 130°–140° C. The autoclave is vented and the contents decanted thereby producing 240 parts of a light yellow liquid. This liquid is stripped at a temperature of 90° C. and a pressure of 10 millimeters of mercury thereby yielding the desired liquid product as the residue.

## EXAMPLE C

Using the procedure of Example B, 136 parts of isoprene, 172 parts of methyl acrylate, and 0.9 part of hydroquinone are converted to the isoprenemethyl acrylate adduct.

## EXAMPLE D

Following the procedure of Example B, 104 parts of liquified butadiene, 166 parts of methyl acrylate, and 1 part of hydroquinone are charged to the rocking autoclave and heated to 130°–135° for 14 hours. The product is subsequently detracted and stripped yielding 237 parts of the adduct.

## EXAMPLE E

The adduct of isoprene and methyl methacrylate is prepared by reacting 745 parts of isoprene with 1095 parts of methyl methacrylate in the presence of 5.4 parts of hydroquinone in the rocking autoclave following the procedure of Example B above. 1490 parts of the adduct is recovered.

## EXAMPLE F

The adduct of butadiene and dibutyl maleate (810 parts) is prepared by reacting 915 parts of dibutyl maleate, 216 parts of liquified butadiene, and 3.4 parts of hydroquinone in the rocking autoclave according to the technique of Example B.

## EXAMPLE G

A reaction mixture comprising 378 parts of butadiene, 778 parts of N-vinylpyrrolidone, and 3.5 parts of hydroquinone is added to a rocking autoclave previously chilled to –35° C. The autoclave is then heated to a temperature of 130°–140° C. for about 15 hours. After venting, decanting, and stripping the reaction mass, 75 parts of the desired adduct are obtained.

## EXAMPLE H

Following the technique of Example B, 270 parts of liquified butadiene, 1060 parts of isodecyl acrylate, and 4 parts of hydroquinone are reacted in the rocking autoclave at a temperature of 130°–140° C. for about 11 hours. After decanting the stripping, 1136 parts of the adduct are recovered.

## EXAMPLE I

Following the stone general procedure of Example A, 132 parts (2 moles) of cyclopentadiene, 256 parts (2 moles) of butyl acrylate, and 12.8 parts of aluminum chloride are reacted to produce the desired adduct. The butyl acrylate and the aluminum chloride are first added to a two-liter flask fitted with stirrer and reflux condenser. While heating reaction mass to a temperature within the range of 59°–52° C., the cyclopentadiene is added to the flask over a 0.5-hour period. Thereafter the reaction mass is heated for about 7.5 hours at a temperature of 95°–100° C. The product is washed with a solution containing 400 parts of water and 100 parts of concentrated hydrochloric acid and the aqueous layer is discarded. Thereafter, 1500 parts of benzene are added to the reaction mass and the benzene solution is washed with 300 parts of water and the aqueous phase removed. The benzene is removed by distillation and the residue stripped at 0.2 parts of mercury to recover the adduct as a distillate.

## EXAMPLE J

Following the technique of Example B, the adduct of butadiene and allyl chloride is prepared using two moles of each reactant.

One-hundred thirty-nine parts (1 mole) of the adduct of butadiene and methyl acrylate is transesterified with 158 parts (1 mole) of decyl alcohol. The reactants are added to a reaction flask and 3 parts of sodium methoxide are added. Thereafter, the reaction mixture is heated at a temperature of 190°–200° C. for a period of 7 hours. The reaction mass is washed with a 10% sodium hydroxide solution and then 250 parts of naphtha is added. The naphtha solution is washed with water. At the completion of the washing, 150 parts of toluene are added and the reaction mass is stripped at 150° C. under pressure of 28 parts of mercury. A dark-brown fluid product (225 parts) is recovered. This product is fractionated under reduced pressure resulting in the recovery of 178 parts of the product boiling in the range of 130°–133° C. at a pressure of 0.45 to 0.6 parts of mercury.

## EXAMPLE L

The general procedure of Example A is repeated except that only 270 parts (5 moles) of butadiene is included in the reaction mixture.

The second sulfurized compositions are readily prepared by heating a mixture of sulfur and at least one of the Diels-Alder adducts of the types discussed herein-

above at a temperature within the range of from about 100° C. to just below the decomposition temperature of the Diels-Alder adducts. Temperatures within the range of about 100° to about 200° C. will normally be used. This reaction results in a mixture of products, some of which have been identified. In the compounds of known structure, the sulfur reacts with the substituted unsaturated cycloaliphatic reactants at a double bond in the nucleus of the unsaturated reactant.

The molar ratio of sulfur to Diels-Alder adduct used in the preparation of the sulfur-containing composition is from about 1:2 up to about 4:1. Generally, the molar ratio of sulfur to Diels-Alder adduct will be from about 1:1 to about 4:1 and preferably about 2:1 to about 4:1 based on the presence of one ethylenically unsaturated bond in the cycloaliphatic nucleus. If there are additional unsaturated bonds in the cycloaliphatic nucleus, the ratio of sulfur may be increased.

The reaction can be conducted in the presence of 20 suitable inert organic solvents such as mineral oils, alkanes of 7 to 18 carbons, etc., although no solvent is generally necessary. After completion of the reaction, the reaction mass can be filtered and/or subjected to other conventional purification techniques. There is no need to separate the various sulfur-containing products as they can be employed in the form of a reaction mixture comprising the compounds of known and unknown structure.

As hydrogen sulfide is an undesirable contaminant, it is advantageous to employ standard procedures for assisting in the removal of the H<sub>2</sub>S from the products. Blowing with steam, alcohols, air, or nitrogen gas assists in the removal of H<sub>2</sub>S as does heating at reduced pressures with or without the blowing.

The following examples illustrate the preparation of the second sulfurized composition.

#### EXAMPLE (D)(12)-11

To 255 parts (1.65 moles) of the isoprene methacrylate adduct of Example C heated to a temperature of 110°-120° C., there are added 53 parts (1.65 moles) of sulfur flowers over a 45-minute period. The heating is continued for 4.5 hours at a temperature in the range of 130°-160° C. After cooling to room temperature, the reaction mixture is filtered through a medium sintered glass funnel. The filtrate consists of 301 parts of the desired second sulfurized composition.

#### EXAMPLE (D)(12)-15

A mixture of 1703 parts (9.4 moles) of a butyl acrylate-butadiene adduct prepared as in Example L, 280 parts (8.8 moles) of sulfur and 17 parts of triphenyl phosphite is prepared in a reaction vessel and heated gradually over 2 hours to a temperature of about 185° C. while stirring and sweeping with nitrogen. The reaction is exothermic near 160°-170° C., and the mixture is maintained at about 185° C. for 3 hours. The mixture is cooled to 90° C. over a period of 2 hours and filtered using a filter aid. The filtrate is the desired second sulfurized composition containing 14.0% sulfur.

#### EXAMPLE (D)(12)-16

The procedure of Example (D)(12)-15 is repeated except that the triphenyl phosphite is omitted from the reaction mixture.

#### EXAMPLE (D)(12)-17

The procedure of Example (D)(12)-15 is repeated except that the triphenyl phosphite is replaced by 2.0 parts of triallyl amine as sulfurization catalyst.

#### EXAMPLE (D)(12)-18

A mixture of 547 parts of a butyl acrylatebutadiene adduct prepared as in Example L and 5.5 parts of triphenyl phosphite is prepared in a reaction vessel and heated with stirring to a temperature of about 50° C. whereupon 94 parts of sulfur are added over a period of 30 minutes. The mixture is heated to 150° C. in 3 hours while sweeping with nitrogen. The mixture then is heated to about 185° C. in approximately one hour. The reaction is exothermic and the temperature is maintained at about 185° C. by using a cold water jacket for a period of about 5 hours. At this time, the contents of the reaction vessel are cooled to 85° C. and 33 parts of mineral oil are added. The mixture is filtered at this temperature, and the filtrate is the desired second sulfurized composition wherein the sulfur to adduct ratio is 0.98/1.

#### EXAMPLE (D)(12)-19

The general procedure of Example (D)(12)-8 with the exception that the triphenyl phosphite is not included in the reaction mixture.

#### EXAMPLE (D)(12)-20

A mixture of 500 parts (2.7 moles) of a butyl acrylatebutadiene adduct prepared as in Example L and 109 parts (3.43 moles) of sulfur is prepared and heated to 180° C. and maintained at a temperature of about 180°-190° C. for about 6.5 hours. The mixture is cooled while sweeping with a nitrogen gas to remove hydrogen sulfide odor. The reaction mixture is filtered and the filtrate is the desired second sulfurized composition containing 15.8% sulfur.

#### Example (D)(12)-21

A mixture of 728 parts (4.0 moles) of a butyl acrylatebutadiene adduct prepared as in Example L, 218 parts (6.8 moles) of sulfur, and 7 parts of triphenyl phosphite is prepared and heated with stirring to a temperature of about 181° C. over a period of 1.3 hours. The mixture is maintained under a nitrogen purge at a temperature of 181°-187° C. for 3 hours. After allowing the material to cool to about 85° C. over a period of 1.4 hours, the mixture is filtered using a filter aid, and the filtrate is the desired second sulfurized composition containing 23.1% sulfur.

It has been found that, if the second sulfurized composition is treated with an aqueous solution of sodium sulfide containing 5% to about 75% by weight Na<sub>2</sub>S, the treated product may exhibit less of a tendency to darken freshly polished copper metal.

Treatment involves the mixing together the second sulfurized composition and the sodium sulfide solution for a period of time sufficient for any unreacted sulfur to be scavenged, usually a period of a few minutes to several hours depending on the amount of unreacted sulfur, the quantity and the concentration of the sodium sulfide solution. The temperature is not critical but normally will be in the range of about 20° C. to about 100° C. After the treatment, the resulting aqueous phase is separated from the organic phase by conventional techniques, i.e., decantation, etc. Other alkali metal sulfides,

M2Sx where M is an alkali metal and x is 1, 2, or 3 may be used to scavenge unreacted sulfur but those where x is greater than 1 are not nearly as effective. Sodium sulfide solutions are preferred for reasons of economy and effectiveness. This procedure is described in more detail in U.S. Pat. No. 3,498,915.

It has also been determined that treatment of the second sulfurized composition with solid, insoluble acidic materials such as acidified clays or acidic resins and thereafter filtering the sulfurized reaction mass improves the product with respect to its color and solubility characteristics. Such treatment comprises thoroughly mixing the reaction mixture with from about 0.1% to about 10% by weight of the solid acidic material at a temperature of about 25°-150° C. and subsequently filtering the product.

In order to remove the last traces of impurities from the second sulfurized composition reaction mixture, particularly when the adduct employed was prepared using a Lewis acid catalyst, (e.g., Al Cl<sub>3</sub>) it is sometimes desirable to add an organic inert solvent to the liquid reaction product and, after thorough mixing, to refilter the material. Subsequently the solvent is stripped from the second sulfurized composition. Suitable solvents include solvents of the type mentioned hereinabove 25 such as benzene, toluene, the higher alkanes, etc. A particularly useful class of solvents are the textile spirits.

In addition, other conventional purification techniques can be advantageously employed in purifying sulfurized products used in this invention. For example, commercial filter aids can be added to the materials prior to filtration to increase the efficiency of the filtration. Filtering through diatomaceous earth is particularly useful where the use contemplated requires the removal of substantially all solid materials. However, such expedients are well known to those skilled in the art and require no elaborate discussion herein.

(D)(13) The Viscosity Index Improver

Viscosity Index or "V.I." is an arbitrary number which indicates the resistance of a lubricant to viscosity change with temperature. The Dean and Davis viscosity index calculated from the observed viscosities of a lubricant at 40° C. and 100° C. gives V.I. values ranging from 0 or negative values to values of 200 or more. The higher its V.I. value, the greater the resistance of a lubricant to thicken at low temperatures and thin out at high temperatures.

An ideal lubricant for most purposes would possess the same viscosity at all temperatures. All lubricants depart from this ideal, some more than others. For example, lubricating oils derived from highly paraffinic crudes have higher V.I. values than lubricating oils derived from highly naphthenic crudes. This difference was used, in fact, to fix the limits of 0 to 100 on the Dean and Davis scale, these values having been assigned, respectively, to a poor naphthene-base oil and a good paraffin-base oil. The operational advantages offered by a lubricant having a high V.I. include principally less friction due to viscous "drag" at low temperatures as well as reduced lubricant loss and lower wear at high temperatures.

V.I. improvers are chemicals which are added to lubricating oils to make them conform more closely to the ideal lubricant defined above. Although a few non-polymeric substances such as metallic soaps exhibit V.I. improving properties, all commercially important V.I. improvers are oil-soluble organic polymers. Suitable polymers exert a greater thickening effect on oil at high

temperatures than they do at lower temperatures. The end result of such selective thickening is that the oil suffers less viscosity change with changing temperature, i.e., its V.I. is raised. It has been proposed that selective thickening occurs because the polymer molecule assumes a compact, curled form in a poor solvent such as cold oil and an uncurred, high surface area form in a better solvent such as hot oil. In the latter form, it is more highly solvated and exerts its maximum thickening effect on the oil.

Commercial V.I. improvers belong to the following families of polymers:

- (I) Polyisobutenes
- (II) Polymethacrylates, i.e., copolymers of various chain length alkyl methacrylates
- (III) Vinyl acetate-fumaric acid ester copolymers
- (IV) Polyacrylates, i.e., copolymers of various chain length alkyl acrylates

(D)(14) The Aromatic Amine

Component (D)(14) is at least one aromatic amine of the formula



30 wherein R<sup>51</sup> is



and R<sup>52</sup> and R<sup>53</sup> are independently a hydrogen or an alkyl group containing from 1 up to 24 carbon atoms. Preferably R<sup>51</sup> is



and R<sup>52</sup> and R<sup>53</sup> are alkyl groups containing from 4 up to about 20 carbon atoms. In a particularly advantageous embodiment, component (D)(9) comprises an alkylated diphenylamine such as nonylated diphenylamine of the formula



The compositions of this invention, components (A), 60 (B), (C) and (D) may optionally contain

(E) at least one oil selected from the group consisting of

- (1) synthetic ester base oil comprising the reaction of a monocarboxylic acid of the formula



or a dicarboxylic acid of the formula



with an alcohol of the formula  
 $R^{56}(\text{OH})_n$

wherein  $R^{54}$  is a hydrocarbyl group containing from about 4 to about 24 carbon atoms,  $R^{55}$  is hydrogen or a hydrocarbyl group containing from about 4 to about 50 carbon atoms,  $R^{56}$  is a hydrocarbyl group containing from 1 to about 24 carbon atoms,  $m$  is an integer of from 0 to about 6 and  $n$  is an integer of from 1 to about 6;

- (2) a mineral oil;
- (3) a polyalphaolefin and
- (4) a vegetable oil.

(E-1) The Synthetic Ester Base Oil

The synthetic ester base oil comprises the reaction of 20 a monocarboxylic acid of the formula



or a dicarboxylic acid of the formula



with an alcohol of the formula



wherein  $R^{54}$  is a hydrocarbyl group containing from about 4 to about 24 carbon atoms,  $R^{55}$  is hydrogen or a hydrocarbyl group containing from about 4 to about 50 carbon atoms,  $R^{56}$  is a hydrocarbyl group containing from 1 to about 24 carbon atoms,  $m$  is an integer of from 0 to about 6 and  $n$  is an integer of from 1 to about 6.

Useful monocarboxylic acids are the isomeric carboxylic acids of pentanoic, hexanoic, octanoic, nonanoic, decanoic, undecanoic and dodecanoic acids. When  $R^{37}$  is hydrogen, useful dicarboxylic acids are succinic acid, maleic acid, azelaic acid, suberic acid, sebacic acid, fumaric acid and adipic acid. When  $R^{37}$  is a hydrocarbyl group containing from 4 to about 50 carbon atoms, the useful dicarboxylic acids are alkyl succinic acids and alkenyl succinic acids. Alcohols that may be employed are methyl alcohol, ethyl alcohol, butyl alcohol, the isomeric pentyl alcohols, the isomeric hexyl alcohols, dodecyl alcohol, 2-ethylhexyl alcohol, ethylene glycol, diethylene glycol, propylene glycol, neopentyl glycol, pentaerythritol, dipentaerythritol, trimethylolpropane, bis-trimethylolpropane, etc. Specific examples of these esters include dibutyl adipate, di(2-ethylhexyl) sebacate, di-n-hexyl fumarate, dioctyl sebacate, diisoctyl azelate, diisodecyl azelate, dioctylphthalate, didecyl phthalate, dieicosyl sebacate, the 2-ethylhexyl diester of linoleic acid dimer, the complex ester formed by reacting one mole of sebacic acid with two moles tetraethylene glycol and two moles of 2-ethylhexanoic acid, the ester formed by reacting one mole of adipic acid with 2 moles of a 9 carbon alcohol derived from the oxo process of a 1-butene dimer and the like.

A non-exhaustive list of companies that produce synthetic esters and their trade names are BASF as Glis-

sofluid, Ciba-Geigy as Reolube, JCI as Emkarote, Olefina as Radialube and the Emery Group of Henkel Corporation as Emery 2964, 2911, 2960, 2976, 2935, 2971, 2930 and 2957.

5 (E-2) The Mineral Oil

The mineral oils having utility are mineral lubricating oils such as liquid petroleum oils and solvent-treated or acid-treated mineral lubricating oils of the paraffinic, naphthenic or mixed paraffinic-naphthenic types. Also useful are petroleum distillates such as VM&P naphtha and Stoddard solvent. Oils of lubricating viscosity derived from coal or shale are also useful. Synthetic lubricating oils include hydrocarbon oils and halosubstituted hydrocarbon oils such as polymerized and interpolymerized olefins (e.g., polybutylenes, polypropylenes, propyleneisobutylene copolymers, chlorinated polybutylenes, etc.); poly(1-hexenes), poly(1-octenes), poly(1-decenes), etc. and mixtures thereof; alkylbenzenes (e.g., dodecylbenzenes, tetradecylbenzenes, dinonylbenzenes, di-(2-ethylhexyl)benzenes, etc.); polyphenyls (e.g., biphenyls, terphenyls, alkylated polyphenyls, etc.); alkylated diphenyl ethers and alkylated diphenyl sulfides and the derivatives, analogs and homologs thereof and the like.

25 Unrefined, refined and rerefined oils, (as well as mixtures of two or more of any of these) can also be used in the present invention. Unrefined oils are those obtained directly from a natural or synthetic source without further purification treatment. For example, a shale oil obtained directly from retorting operations, a petroleum oil obtained directly from primary distillation or ester oil obtained directly from an esterification process and used without further treatment would be an unrefined oil. Refined oils are similar to the unrefined oils except they have been further treated in one or more purification steps to improve one or more properties. Many such purification techniques are known to those skilled in the art such as solvent extraction, secondary distillation, acid or base extraction, filtration, percolation, etc. Rerefined oils are obtained by processes similar to those used to obtain refined oils applied to refined oils which have been already used in service. Such rerefined oils are also known as reclaimed or reprocessed oils and often are additionally processed by techniques directed to removal of spent additives and oil breakdown products.

30 (E-3) The Polyalpha Olefins

50 Polyalpha olefins such as alkylene oxide polymers and interpolymers and derivatives thereof where the terminal hydroxyl groups have been modified by esterification, etherification, etc., constitute another class of oils that can be used. These are exemplified by the oils prepared through polymerization of ethylene oxide or propylene oxide, the alkyl and aryl ethers of these polyoxyalkylene polymers (e.g., methylpolyisopropylene glycol ether having an average molecular weight of about 1000, diphenyl ether of polyethylene glycol having a molecular weight of about 500-1000, diethyl ether 55 of polypropylene glycol having a molecular weight of about 1000-1500, etc.) or mono- and polycarboxylic esters thereof, for example, the acetic acid esters, mixed 60 C<sub>3</sub>-C<sub>8</sub> fatty acid esters, or the C<sub>13</sub> Oxo acid diester of tetraethyleneglycol.

65 (E-4) The Vegetable Oils

Vegetable oils having utility in this invention are those vegetable oils obtained without genetic modification, i.e., their monounsaturation content (as oleic acid)

is below 60 percent. Vegetable oils having utility are canola oil, peanut oil, palm oil, corn oil, soybean oil, sunflower oil, cottonseed oil, safflower oil and coconut oil.

When the composition of this invention comprises components (A), (B), (C) and (D), the following states the ranges of these components in parts by weight:

| COMPONENT | GENERALLY | PREFERRED | MOST PREFERRED | 10 |
|-----------|-----------|-----------|----------------|----|
| (A)       | 40-95     | 40-80     | 40-70          |    |
| (B)       | 10-40     | 15-40     | 15-35          |    |
| (C)       | 0.1-20    | 0.1-10    | 0.5-5          |    |
| (D)       | 0.001-1.0 | 0.01-0.5  | 0.01-0.1       |    |

When the composition of this invention comprises components (A), (B), (C), (D) and (E), the following states the ranges of these components in parts by weight:

| COMPONENT | GENERALLY | PREFERRED | MOST PREFERRED | 20 |
|-----------|-----------|-----------|----------------|----|
| (A)       | 40-95     | 40-80     | 40-70          |    |
| (B)       | 10-40     | 15-40     | 15-35          |    |
| (C)       | 0.1-20    | 0.1-10    | 0.5-5          |    |
| (D)       | 0.001-1.0 | 0.01-0.5  | 0.01-0.1       |    |
| (E)       | 5-25      | 5-20      | 10-20          |    |

The components of this invention are blended together according to the above ranges to effect solution. The following Table I outlines examples so as to provide those of ordinary skill in the art with a complete disclosure and description on how to make the composition of this invention and is not intended to limit the scope of what the inventor regards as his invention. All parts are by weight.

TABLE II

| EXAMPLE | (A)                 | (B)                     | (C)                    |  |
|---------|---------------------|-------------------------|------------------------|--|
| 1       | 100 parts Sunyl 80  |                         |                        |  |
| 2       |                     | 100 parts Example B-1   |                        |  |
| 3       | 66.4 parts Sunyl 80 | 16.6 parts Example B-1  | 2 parts TLA 233        |  |
| 4       | 67 parts Sunyl 80   | 16.75 parts Example B-1 | 1.25 parts Example C-8 |  |
| 5       | 57.4 parts Sunyl 80 | 24.6 parts Example B-1  | 3 parts Example C-8    |  |
| 6       | 58.1 parts Sunyl 80 | 24.9 parts Example B-1  | 2 parts Acryloid 1267  |  |
| 7       | 49.5 parts Sunyl 80 | 33 parts Example B-1    | 2.5 parts Example C-9  |  |

  

| EXAMPLE<br>(D) |                              | 100° C.       |      |     |     | Pour<br>Point | Freeze<br>Point |
|----------------|------------------------------|---------------|------|-----|-----|---------------|-----------------|
|                |                              | 40° C.<br>VIS | VIS  | VI  |     |               |                 |
| 1              |                              | 39.52         | 8.65 | 206 | -12 | -14.6         |                 |
| 2              |                              | 4.62          | 1.79 | —   | -12 | -13.6         |                 |
| 3              | 7.5 parts Example (D)(10)a-1 | 46.94         | 9.99 | 207 | -18 | -20.2         |                 |
|                | 7.5 parts Example (D)(10)b-2 |               |      |     |     |               |                 |
| 4              | 7.5 parts Example (D)(10)a-1 | 45.48         | 9.46 | 198 | -27 | -27.2         |                 |
|                | 7.5 parts Example (D)(10)b-2 |               |      |     |     |               |                 |
| 5              | 7.5 parts Example (D)(10)a-1 | 44.39         | 9.72 | 212 | -33 | -33.6         |                 |
|                | 7.5 parts Example (D)(10)b-2 |               |      |     |     |               |                 |
| 6              | 7.5 parts Example (D)(10)a-1 | 36.90         | 8.23 | 208 | -33 | -35.8         |                 |
|                | 7.5 parts Example (D)(10)b-2 |               |      |     |     |               |                 |
| 7              | 7.5 parts Example (D)(10)a-1 | 36.30         | 8.68 | 231 | -30 | -32.2         |                 |
|                | 7.5 parts Example (D)(10)b-2 |               |      |     |     |               |                 |

While the invention has been explained in relation to its preferred embodiments, it is to be understood that various modifications thereof will become apparent to those skilled in the art upon reading the specification. Therefore, it is to be understood that the invention disclosed herein is intended to cover such modifications as fall within the scope of the appended claims.

What is claimed is:

1. A composition, comprising;
- (A) at least one vegetable or synthetic triglyceride oil of the formula



wherein R<sup>1</sup>, R<sup>2</sup> and R<sup>3</sup> are aliphatic hydrocarbyl groups having at least 60 percent monounsaturated character and containing from about 6 to about 24 carbon atoms;

- (B) esters from the transesterification of at least one animal or vegetable oil triglyceride of the formula



with an alcohol or phenol R<sup>4</sup>OH wherein R<sup>1</sup>, R<sup>2</sup> and R<sup>3</sup> are aliphatic groups containing from about 6 to about 24 carbon atoms and R<sup>4</sup> is an aliphatic group containing from 1 to about 10 carbon atoms or an aromatic or substituted aromatic group containing from 6 to about 50 carbon atoms;

- (C) a pour point depressant;

(D) at least one performance additive selected from the group consisting of

- (1) at least one alkyl phenol of the formula



5

wherein R¹¹ is an alkyl group containing from 1 up to about 24 carbon atoms and a is an integer of from 1 up to 5;

(2) a benzotriazole of the formula



15

wherein R¹² is hydrogen or an alkyl group of 1 up to about 24 carbon atoms;

(3) a phosphatide of the formula



25

wherein R¹³ and R¹⁴ are aliphatic hydrocarbyl groups containing from 8 to about 24 carbon atoms, and G is selected from the group consisting of hydrogen;



40

(4) a thiocarbamate of the formula



45

wherein R¹⁵ is an alkyl group containing from 1 to about 24 carbon atoms, phenyl or alkyl phenyl wherein the alkyl group contains from 1 to about 18 carbon atoms, R¹⁶ and R¹⁷ are hydrogen or an alkyl group containing from 1 to about 6 carbon atoms, with the proviso that R¹⁶ and R¹⁷ are not both hydrogen;

(5) citric acid and derivatives of citric acid of the formula



60

65

wherein R¹⁸, R¹⁹ and R²⁰ are independently hydrogen or aliphatic hydrocarbyl groups containing from 1 to about 12 carbon atoms, or an aromatic or substituted aromatic groups containing from 6 to about 50 carbon atoms with the proviso that at least one of R¹⁷, R¹⁸ and R¹⁹ is an aliphatic hydrocarbyl group;

(6) a coupled phosphorus-containing amide of the formula



wherein X¹, X² and X³ independently is oxygen or sulfur;

wherein R²¹ and R²², independently is a hydrocarbyl, a hydrocarbyl-based oxy, the hydrocarbyl portions of which contain 6 to about 22 carbon atoms, or a hydrocarbyl-based thio, having from 4 to about 34 carbon atoms;

wherein R²³, R²⁴, R²⁵ and R²⁶, independently is hydrogen, or an alkyl having from 1 to about 22 carbon atoms, or an aromatic, an alkyl-substituted aromatic or an aromatic-substituted alkyl having from 6 to about 34 atoms;

wherein n is zero or 1;

wherein n' is 2 or 3

wherein R²⁷ is hydrogen; and when n' is 2, R²⁸ is selected from the group consisting of



wherein R is an alkyl moiety, in the form of alkylene or alkylidene containing from 1 to 12 carbon atoms and R' is an alkyl moiety, alkylene, alkylidene or carboxyl containing 1 to 60 carbon atoms and when n' is 3, R²⁷ is



(7) a methylacrylate derivative formed by the reaction of equal molar amounts of a phosphorus acid of the formula



with methylacrylate wherein X¹ and X² are oxygen or sulfur and R²⁹ and R³⁰ are each independently a hydrocarbyl, a hydrocarbyl-based thio or preferably a hydrocarbyl-based oxy group wherein the hydrocarbyl portion contains from 1

to about 30 carbon atoms and remaining acidity is neutralized with 1 mole propylene oxide for each 20-25 moles of phosphorus acid;

- (8) a metal overbased composition;
- (9) a carboxylic dispersant composition;
- (10) a nitrogen-containing organic composition comprising
  - (a) an acylated, nitrogen containing compound having a substituent of at least 10 aliphatic carbon atoms made by reacting a carboxylic acylating agent with at least one amino compound containing at least one —NH group, said acylating agent being linked to said amino compound through an imido, amido, amidine or acyloxy ammonium linkage; and
  - (b) at least one amino phenol of the general formula



wherein  $\text{R}^{37}$  is a substantially saturated, hydrocarbon-based substituent of at least 10 aliphatic carbon atoms; a, b and c are each independently an integer of one up to three times the number of aromatic nuclei present in Ar with the proviso that the sum of a, b and c does not exceed the unsaturated valences of Ar; and Ar is an aromatic moiety having 0-3 optional substituents selected from the group consisting of lower alkyl, lower alkoxy, nitro, halo or combinations of two or more of said substituents;

- (11) a zinc salt of the formula



wherein  $\text{R}^{43}$  and  $\text{R}^{44}$  are independently hydrocarbyl groups containing from about 3 to about 20 carbon atoms;

- (12) a sulfurized composition wherein the sulfurized composition is a sulfurized olefin prepared by reacting an olefin with sulfur or sulfur halide complex;
- (13) at least one viscosity index improver; and
- (14) at least one aromatic amine of the formula



wherein  $\text{R}^{51}$  is



and  $\text{R}^{52}$  and  $\text{R}^{53}$  are independently a hydrogen or an alkyl group containing from 1 up to about 24 carbon atoms; and optionally

- (E) at least one oil selected from the group consisting of
  - (1) synthetic ester base oil comprising the reaction of a monocarboxylic acid of the formula



or a dicarboxylic acid of the formula



with an alcohol of the formula



wherein  $\text{R}^{54}$  is a hydrocarbyl group containing from about 4 to about 24 carbon atoms,  $\text{R}^{55}$  is hydrogen or a hydrocarbyl group containing from about 4 to about 50 carbon atoms,  $\text{R}^{56}$  is a hydrocarbyl group containing from 1 to about 24 carbon atoms, m is an integer of from 0 to about 6 and n is an integer of from 1 to about 6;

- (2) a mineral oil;
- (3) a polyalphaolefin; and
- (4) a vegetable oil.

- 2. The composition of claim 1 wherein the triglyceride for (A) or (B) is a vegetable oil triglyceride.

- 3. The composition of claim 2 wherein the vegetable oil triglyceride is an ester of at least one straight chain fatty acid and glycerol wherein the fatty acid contains from about 8 to about 22 carbon atoms.

- 4. The composition of claim 3 wherein the triglyceride is at least 70 percent monounsaturated.

- 5. The composition of claim 4 wherein the triglyceride is at least 80 percent monounsaturated.

- 6. The composition of claim 5 wherein the monounsaturated character is due to an oleic acid residue.

- 7. The composition of claim 2 wherein the vegetable oil triglyceride comprises sunflower oil, safflower oil, corn oil, soybean oil, rapeseed oil, meadowfoam oil or genetically modified sunflower oil, safflower oil, corn oil, soybean oil, rapeseed oil or meadowfoam oil.

- 8. The composition of claim 1 whereto  $\text{R}^4$  contains from about 1 to about 6 carbon atoms.

- 9. The composition of claim 1 wherein the transesterification of (B) is carried out in the presence of a catalyst comprising alkali or alkaline earth metal alkoxides.

- 10. The composition of claim 1 wherein the transesterification is carried out at a temperature of ambient up to the decomposition temperature of any reactant or product.

- 11. The composition of claim 1 wherein the pour point depressant is a mixed ester characterized by low-temperature modifying properties of an ester of a carboxy-containing interpolymer, said interpolymer having a reduced specific viscosity of from about 0.05 to about 2 and being derived from at least two monomers, one of said monomers being a low molecular weight aliphatic olefin, styrene or a substituted styrene wherein the substituent is a hydrocarbyl group containing from 1 up to about 18 carbon atoms, and the other of said

monomers being an alpha, beta-unsaturated aliphatic acid, anhydride or ester thereof, said ester being substantially free of titratable acidity and being characterized by the presence within its polymeric structure of at least one of each of three pendant polar groups which are derived from the carboxy groups of said ester:

- (A) a relatively high molecular weight carboxylic ester group, said carboxylic ester group having at least 8 aliphatic carbon atoms in the ester radical,
- (B) a relatively low molecular weight carboxylic ester group having no more than 7 aliphatic carbon atoms in the ester radical, wherein the molar ratio of (A):(B) of the pour point depressant is (1-20):1, and optionally
- (C) a carbonyl-amino group derived from an amino compound having one primary or secondary amino group, wherein the molar ratio of (A):(B):(C) of the pour point depressant is (50-100):(5-50):(0.1-15).

12. The composition of claim 11 wherein said mixed ester of the interpolymer is characterized by low-temperature modifying properties of an ester of a carboxy-containing interpolymer, said interpolymer having a reduced specific viscosity of from about 0.05 to about 2 and being derived from at least two monomers, the one being ethylene, propylene, isobutene, styrene or substituted styrene wherein the substituent is a hydrocarbyl group containing from 1 up to about 18 carbon atoms and the other of said monomers being maleic acid or anhydride, itaconic acid or anhydride or acrylic acid or ester, said ester being substantially free of titratable acidity and being characterized by the presence within its polymeric structure of at least one of each of three pendant polar groups which are derived from the carboxy groups of said ester:

- (A) a relatively high molecular weight carboxylic ester group, said carboxylic ester group having at least 8 aliphatic carbon atoms in the ester radical,
- (B) a relatively low molecular weight carboxylic ester group having no more than 7 aliphatic carbon atoms in the ester radical, wherein the molar ratio of (A):(B) of the pour point depressant is (1-20):1, and optionally
- (C) a carbonyl-amino group derived from an amino compound having one primary or secondary amino radical, wherein the molar ratio of (A):(B):(C) of the pour point depressant is (50-100):(5-50):(0.1-15).

13. The composition of claim 11 wherein the molar ratio of (A):(B) of the pour point depressant is (1-10):1.

14. The composition of claim 11 wherein the molar ratio of (A):(B):(C) of the pour point depressant is (70-85):(15-30):(3-4).

15. The composition of claim 11 wherein the interpolymer is a styrene-maleic anhydride interpolymer having a reduced specific viscosity of from about 0.1 to about 1.

16. The composition of claim 11 wherein the relatively high molecular weight carboxylic ester group of (A) has from 8 to 24 aliphatic carbon atoms, the relatively low molecular weight carboxylic ester group of (B) has from 3 to 5 carbon atoms and the carbonyl-amino group of (C) is derived from a primary-aminoalkyl-substituted tertiary amine.

17. The composition of claim 11 wherein the carboxy-containing interpolymer is a terpolymer of one molar proportion of styrene, one molar proportion of maleic anhydride, and less than about 0.3 molar proportion of a vinyl monomer.

18. The composition of claim 11 wherein said low molecular weight aliphatic olefin of said nitrogen-containing ester is selected from the group consisting of ethylene, propylene or isobutene.

19. The composition of claim 1 wherein the pour point depressant is an acrylate polymer of the formula



wherein R<sup>5</sup> is hydrogen or a lower alkyl group containing from 1 to about 4 carbon atoms, R<sup>6</sup> is a mixture of alkyl, cycloalkyl or aromatic groups containing from about 4 to about 24 carbon atoms, and x is an integer providing a weight average molecular weight (M<sub>w</sub>) to the acrylate polymer of about 5000 to about 1,000,000.

20. The composition of claim 19 wherein R<sup>5</sup> is a methyl group.

21. The composition of claim 19 wherein the molecular weight of the polymer is from about 50,000 to about 500,000.

22. The composition of claim 1 wherein the pour point depressant is a mixture of compounds having the general structural formula



wherein the Ar, Ar' and Ar'' are independently an aromatic moiety containing 1 to 3 aromatic rings and the mixture includes compounds wherein moieties are present with 0 substituents, 1 substituent, 2 substituents and 3 substituents, R<sup>7</sup> and R<sup>8</sup> are independently an alkylene containing about 1 to 100 carbon atoms, and n is 0 to 1000.

23. The mixture as claimed in claim 22, wherein compounds are present in the mixture wherein the aromatic moieties are naphthalene, the olefin contains about 16 to 18 carbon atoms and the chlorinated hydrocarbon contains about 20 to 26 carbon atoms.

24. The mixture as claimed in claim 22 including compounds having a molecular weight ranging from about 300 to about 10,000.

25. The mixture as claimed in claim 22 including compounds having a molecular weight ranging from about 300 to about 300,000.

26. The composition of claim 1 wherein the pour point depressant is a nitrogen containing polymer prepared by polymerizing an acrylate ester monomer of the formula



wherein R<sup>9</sup> is hydrogen or an alkyl group containing from 1 to about 4 carbon atoms and R<sup>10</sup> is an alkyl, cycloalkyl or aromatic group containing from 4 to about 24 carbon atoms with a nitrogen-containing monomer at from 0.001-1.0 moles of the nitrogen containing monomer for each mole of the acrylate ester monomer.

27. The composition of claim 26 wherein the nitrogen-containing monomer is selected from the group consisting of 4-vinylpyridine, 2-vinylpyridine, 2-N-morpholinoethyl methacrylate, N,N-dimethylaminoethyl

methacrylate and N,N-dimethylaminopropyl methacrylate.

28. The composition of claim 1 wherein within (D)(1) a is 2 and R<sup>11</sup> contains from 1 up to about 8 carbon atoms.

29. The composition of claim 28 wherein the alkyl phenol is of the formula



wherein R<sup>11</sup> is t-butyl.

30. The composition of claim 1 wherein within (D)(2) R<sup>12</sup> is hydrogen or an alkyl group containing from 1 up to about 8 carbon atoms.

31. The composition of claim 1 wherein within (D)(2) R<sup>12</sup> is a methyl group.

32. The composition of claim 1 wherein within (D)(7) X<sup>1</sup> and X<sup>2</sup> are sulfur and R<sup>29</sup> and R<sup>30</sup> are hydrocarbyl-based oxy groups wherein the hydrocarbyl group contains from 1 to 12 carbon atoms.

33. The composition of claim 1 wherein within (D)(8) the metal overbased composition is selected from the group consisting of

- (a) a metal overbased phenate derived from the reaction of an alkylated phenol wherein the alkyl group has at least 6 aliphatic carbon atoms optionally reacted with formaldehyde or a sulfurization agent or mixtures thereof,
- (b) a metal overbased sulfonate derived from an alkylated aryl sulfonic acid wherein the alkyl group has at least 15 aliphatic carbon atoms and
- (c) a metal overbased carboxylate derived from fatty acids having at least 8 aliphatic carbon atoms.

34. The composition of claim 33 wherein the metal is an alkali or alkaline earth metal.

35. The composition of claim 33 wherein the alkaline earth metal is calcium or magnesium.

36. The composition of claim 33 wherein the alkali metal is sodium.

37. The composition of claim 33 wherein the metal overbased composition is treated with a borating agent.

38. The composition of claim 1 wherein within (D)(9) the carboxylic dispersant composition comprises the reaction of a hydrocarbon substituted succinic acid-producing compound with at least about one-half equivalent, per equivalent of acid producing compound, of an organic hydroxy compound or an amine containing at least one hydrogen attached to a nitrogen atom, or a mixture of said hydroxy compound and amine.

39. The composition of claim 38 wherein within (D)(9) the succinic acid-producing compound contains an average of at least about 50 aliphatic carbon atoms in the substituent.

40. The composition of claim 38 wherein within (D)(9) the succinic acid producing compound is selected from the group consisting of succinic acids, anhydrides, esters and halides.

41. The composition of claim 38 wherein within (D)(9) the hydrocarbon substituent of the succinic acid producing compound is derived from a polyolefin having an Mn value within the range of from about 700 to about 10,000.

42. The composition of claim 38 wherein within (D)(9) the amine reacted with the succinic acid producing compound is characterized by the formula

5 R<sup>35</sup>R<sup>36</sup>NH

wherein R<sup>35</sup> and R<sup>36</sup> are each independently hydrogen, or hydrocarbon, amino-substituted hydrocarbon, hydroxy-substituted hydrocarbon, alkoxy-substituted hydrocarbon, amino, carbamyl, thiocarbamyl, guanyl, and acylimidoyl groups provided that only one of R<sup>35</sup> and R<sup>36</sup> may be hydrogen.

43. The composition of claim 38 wherein within (D)(9) the amine reacted with the succinic acid producing compound is a polyamine.

44. The composition of claim 1 wherein within (D)(10)(a) the amino compound is an alkylene polyamine of the general formula



Formula IX

wherein U is an alkylene group of 2 to 10 carbon atoms; 25 each R<sup>38</sup> is independently a hydrogen atom, a lower alkyl group or a lower hydroxy alkyl group, with the proviso that at least one R<sup>38</sup> is a hydrogen atom, and n is 1 to 10.

45. The composition of claim 44 wherein within (D)(10)(a) the acylating agent is a mono- or polycarboxylic acid, or reactant equivalent thereof, containing an aliphatic hydrocarbyl substituent of at least about 30 carbon atoms.

46. The composition of claim 45 wherein within (D)(10)(a) the substituent is made from a homo- or interpolymer of a C<sub>2</sub>-10 1-monoolefin or mixtures thereof.

47. The composition of claim 46 wherein within (D)(10)(a) the homo- or interpolymer is of ethylene, propylene, 1-butene, 2-butene, isobutene or mixtures thereof.

48. The composition of claim 44 wherein within (D)(10)(a) the acylating agent is at least one mono-carboxylic acid, or reactant equivalent thereof, having from 12 to 30 carbon atoms.

49. The composition of claim 48 wherein within (D)(10)(a) the acylating agent is a mixture of fatty monocarboxylic acids, or reactant equivalent thereof, having straight and branched carbon chains.

50. The composition of claim 49 wherein within (D)(10)(a) the amino compound is an ethylene, propylene or trimethylene polyamine of at least 2 to about 8 amino groups or mixtures of such polyamines.

51. The composition of claim 1 wherein within (D)(10)(b) R<sup>37</sup> contains up to about 750 carbon atoms

55 and there are no optional substituents attached to Ar.

52. The composition of claim 51 wherein within (D)(10)(b) R<sup>37</sup> is an alkyl or alkenyl group.

53. The composition of claim 1 wherein within (D)(10)(b) R<sup>37</sup> contains about 30 to about 750 aliphatic 60 carbon atoms and is made from a homo- or interpolymer of C<sub>2</sub>-C<sub>10</sub> olefins.

54. The composition of claim 53 wherein within (D)(10)(b) said olefins are selected from the group consisting of ethylene, propylene, butylene and mixtures thereof.

55. The composition of claim 1 wherein within (D)(10)(b) a, b and c are each 1, there are zero optional substituents attached to Ar, and Ar is a benzene nucleus.

56. The composition of claim 55 wherein within (D)(10)(b) R<sup>37</sup> is an alkyl or alkenyl group of at least about 30 carbon atoms and up to about 750 carbon atoms and is derived from a homo or interpolymer of C<sub>2</sub>-C<sub>10</sub> 1-monoolefins.

57. The composition of claim 1 wherein within (D)(10)(b) the amino phenol is of the formula



wherein R<sup>39</sup> is a substantially saturated hydrocarbon-based substituent having an average of from about 30 to about 400 aliphatic carbon atoms, R<sup>40</sup> is a member selected from the group consisting of lower alkyl, lower alkoxy, nitro, and halo; and z is zero or one.

58. The composition of claim 57 wherein within (D)(10)(b) R<sup>39</sup> is a purely hydrocarbyl aliphatic group of at least about 50 carbon atoms and is made from a polymer or interpolymer of an olefin selected from the group consisting of C<sub>2</sub>-<sub>10</sub> 1-monoolefins and mixtures thereof.

59. The composition of claim 58 wherein within (D)(10)(b) z is zero.

60. The composition of claim 1 wherein within (D)(12) the olefin is an alkylene compound containing one double bond and 2 to 50 carbon atoms, and the sulfur halide is a sulfur chloride.

61. The composition of claim 1 wherein within (D)(12) the olefin is a mixture of olefins containing isobutene and the sulfur halide is selected from the group consisting of sulfur monochloride, sulfur dichloride and mixtures thereof; the protic solvent is selected from the group consisting of water, alcohols, carboxylic

acids and combination thereof; and the metal ions are sodium sulfide/sodium hydrosulfide mixture derived from hydrocarbon purification process streams and sodium hydroxide.

5 62. The composition of claim 1 wherein within (D)(12) the sodium sulfide/sodium hydrosulfide mixture is derived from hydrocarbon purification process streams.

10 63. The composition of claim 1 wherein within (D)(12) the olefin contains one double bond and 2 to 50 carbon atoms and the sulfur halide is a sulfur chloride.

15 64. The composition of claim 63 wherein within (D)(12) the olefin is isobutene, the sulfur halide is sulfur monochloride, and the protic solvent is a water-isopropyl alcohol mixture.

65. The composition of claim 1 wherein within (D)(12) the molar ratio of sulfur to adduct is from about 2:1 to about 4:1.

20 66. The composition of claim 65 wherein within (D)(12) the diene is further characterized in that R<sup>47</sup> and R<sup>48</sup> are hydrogen and R<sup>45</sup>, R<sup>46</sup>, R<sup>49</sup> and R<sup>50</sup> are each independently hydrogen, chloro, or lower alkyl.

67. The composition of claim 62 wherein within (D)(12) the diene is 1,3-butadiene.

68. The composition of claim 1 wherein within (D)(14) R<sup>51</sup> is



35 and R<sup>52</sup> and R<sup>53</sup> are alkyl groups containing from 4 to 18 carbon atoms.

69. The composition of claim 68 wherein within (D)(14) R<sup>52</sup> and R<sup>53</sup> are nonyl groups.

\* \* \* \* \*